



US010281831B2

(12) **United States Patent**  
**Cote et al.**

(10) **Patent No.:** **US 10,281,831 B2**  
(45) **Date of Patent:** **May 7, 2019**

(54) **IMAGING MEMBERS COMPRISING  
CAPPED STRUCTURED ORGANIC FILM  
COMPOSITIONS**

(71) Applicant: **XEROX CORPORATION**, Norwalk, CT (US)

(72) Inventors: **Adrien P. Cote**, Clarkson (CA); **Gregory McGuire**, Oakville (CA); **Richard A. Klenkler**, San Jose, CA (US)

(73) Assignee: **XEROX CORPORATION**, Norwalk, CT (US)

(\*) Notice: Subject to any disclaimer, the term of this patent is extended or adjusted under 35 U.S.C. 154(b) by 17 days.

(21) Appl. No.: **14/636,495**

(22) Filed: **Mar. 3, 2015**

(65) **Prior Publication Data**

US 2016/0259256 A1 Sep. 8, 2016

(51) **Int. Cl.**

**G03G 5/06** (2006.01)  
**G03G 5/05** (2006.01)  
**G03G 5/07** (2006.01)  
**G03G 5/147** (2006.01)

(52) **U.S. Cl.**

CPC ..... **G03G 5/0618** (2013.01); **G03G 5/0539** (2013.01); **G03G 5/0614** (2013.01); **G03G 5/0616** (2013.01); **G03G 5/075** (2013.01); **G03G 5/076** (2013.01); **G03G 5/14726** (2013.01); **G03G 5/14786** (2013.01); **G03G 5/14791** (2013.01); **G03G 5/14795** (2013.01)

(58) **Field of Classification Search**

None

See application file for complete search history.

(56)

**References Cited**

U.S. PATENT DOCUMENTS

|              |         |                 |
|--------------|---------|-----------------|
| 4,265,990 A  | 5/1981  | Stolka et al.   |
| 4,286,033 A  | 8/1981  | Neyhart et al.  |
| 4,291,110 A  | 9/1981  | Lee             |
| 4,338,387 A  | 7/1982  | Hewitt          |
| 4,457,994 A  | 7/1984  | Pai et al.      |
| 4,464,450 A  | 8/1984  | Teuscher        |
| 4,664,995 A  | 5/1987  | Horgan et al.   |
| 4,871,634 A  | 10/1989 | Limburg et al.  |
| 4,921,769 A  | 5/1990  | Yuh et al.      |
| 4,921,773 A  | 5/1990  | Melnyk et al.   |
| 5,455,136 A  | 10/1995 | Yu et al.       |
| 5,702,854 A  | 12/1997 | Schank et al.   |
| 5,853,906 A  | 12/1998 | Hsieh           |
| 5,976,744 A  | 11/1999 | Fuller et al.   |
| 7,177,572 B2 | 2/2007  | DiRubio et al.  |
| 7,202,002 B2 | 4/2007  | Tokarski et al. |
| 7,384,717 B2 | 6/2008  | Dinh et al.     |

(Continued)

OTHER PUBLICATIONS

Cote, et al., U.S. Appl. No. 12/815,688, filed Jun. 15, 2010.

(Continued)

*Primary Examiner* — Joshua D Zimmerman

(74) *Attorney, Agent, or Firm* — Pillsbury Winthrop Shaw Pittman LLP

(57) **ABSTRACT**

An imaging member outer layer comprising a structured organic film comprising a plurality of segments and a plurality of linkers arranged as a covalent organic framework, wherein the structured organic film further includes fluorinated segments and capping units comprising hole transport materials.

**18 Claims, 3 Drawing Sheets**



(56)

**References Cited**

U.S. PATENT DOCUMENTS

|              |     |        |               |             |
|--------------|-----|--------|---------------|-------------|
| 7,416,824    | B2  | 8/2008 | Kondoh et al. |             |
| 2003/0042850 | A1* | 3/2003 | Bertram ..... | B82Y 10/00  |
|              |     |        |               | 313/504     |
| 2012/0040283 | A1* | 2/2012 | Heuft .....   | G03G 5/0589 |
|              |     |        |               | 430/56      |
| 2014/0045108 | A1* | 2/2014 | Vella .....   | G03G 5/0539 |
|              |     |        |               | 430/56      |

OTHER PUBLICATIONS

Cote, et al. U.S. Appl. No. 12/716,706, filed Mar. 3, 2010.  
Heuft, et al., U.S. Appl. No. 12/716,686, filed Mar. 3, 2010.  
Heuft, et al., U.S. Appl. No. 12/716,571, filed Mar. 3, 2010.  
Heuft, et al., U.S. Appl. No. 12/716,524, filed Mar. 3, 2010.  
Cote, et al., U.S. Appl. No. 12/716,449, filed Mar. 3, 2010.  
Heuft, et al., U.S. Appl. No. 12/716,324, filed Mar. 3, 2010.

\* cited by examiner



FIG. 1



FIG. 2



FIG. 3



FIG. 4



FIG. 5

## 1

IMAGING MEMBERS COMPRISING  
CAPPED STRUCTURED ORGANIC FILM  
COMPOSITIONS

## BACKGROUND

The presently disclosed embodiments relate generally to a structured organic film (SOF) comprising a plurality of segments and a plurality of linkers arranged as a covalent organic framework (COF), wherein the SOF comprises capping units. In particular embodiments, the SOF comprises fluorinated segments and the capping units are hole transport molecules. In the present embodiments, the SOF is used for forming the outer layer of an imaging member.

In electrophotography, also known as Xerography, electrophotographic imaging or electrostatographic imaging, the surface of an electrophotographic plate, drum, belt or the like (imaging member or photoreceptor) containing a photoconductive insulating layer on a conductive layer is first uniformly electrostatically charged. The imaging member is then exposed to a pattern of activating electromagnetic radiation, such as light. The radiation selectively dissipates the charge on the illuminated areas of the photoconductive insulating layer while leaving behind an electrostatic latent image on the non-illuminated areas. This electrostatic latent image may then be developed to form a visible image by depositing finely divided electroscopic marking particles on the surface of the photoconductive insulating layer. The resulting visible image may then be transferred from the imaging member directly or indirectly (such as by a transfer or other member) to a print substrate, such as transparency or paper. The imaging process may be repeated many times with reusable imaging members.

Although excellent toner images may be obtained with multilayered belt or drum photoreceptors, it has been found that as more advanced, higher speed electrophotographic copiers, duplicators, and printers are developed, there is a greater demand on print quality. The delicate balance in charging image and bias potentials, and characteristics of the toner and/or developer, must be maintained. This places additional constraints on the quality of photoreceptor manufacturing, and thus on the manufacturing yield.

Imaging members are generally exposed to repetitive electrophotographic cycling, which subjects the exposed charged transport layer or alternative top layer thereof to mechanical abrasion, chemical attack and heat. This repetitive cycling leads to gradual deterioration in the mechanical and electrical characteristics of the exposed charge transport layer. Physical and mechanical damage during prolonged use, especially the formation of surface scratch defects, is among the chief reasons for the failure of belt photoreceptors. Therefore, it is desirable to improve the mechanical robustness of photoreceptors, and particularly, to increase their scratch resistance, thereby prolonging their service life. Additionally, it is desirable to increase resistance to light shock so that image ghosting, background shading, and the like is minimized in prints.

Providing a protective overcoat layer is a conventional means of extending the useful life of photoreceptors. Conventionally, for example, a polymeric anti-scratch and crack overcoat layer has been utilized as a robust overcoat design for extending the lifespan of photoreceptors. However, the conventional overcoat layer formulation exhibits ghosting and background shading in prints. Improving light shock resistance will provide a more stable imaging member resulting in improved print quality.

## 2

Despite the various approaches that have been taken for forming imaging members, there remains a need for improved imaging member design, to provide improved imaging performance and longer lifetime, reduce human and environmental health risks, and the like.

Capped “Structured organic films” (SOFs) described herein are exceptionally chemically and mechanically robust materials that demonstrate many superior properties to conventional photoreceptor materials and increase the photoreceptor life by preventing chemical degradation pathways caused by the xerographic process. Additionally, additives maybe added to improve the morphological properties of the SOF by tuning the SOF to possess desired properties.

15

## SUMMARY OF THE DISCLOSURE

There is provided in embodiments a structured organic film comprising a plurality of segments and a plurality of linkers arranged as a covalent organic framework, wherein at a macroscopic level the covalent organic framework is a film.

In embodiments, there is provided an imaging member comprising: a substrate; a charge generating layer; a charge transport layer; and an optional overcoat layer, wherein an outermost layer of the imaging member comprises a structured organic film (SOF) comprising a plurality of segments and a plurality of linkers arranged as a covalent organic framework (COF), wherein the SOF comprises capping units and further wherein the capping units comprise hole transport molecules.

In further embodiments, there is provided an imaging member comprising: a substrate; a charge generating layer; a charge transport layer; and an optional overcoat layer, wherein an outermost layer of the imaging member comprises a structured organic film (SOF) comprising a plurality of segments including at least a first fluorinated segment and a plurality of linkers arranged as a covalent organic framework (COF), wherein the SOF further comprises capping units that are hole transport molecules further wherein a capping unit loading is greater than 5% by weight of the total weight of the SOF.

In yet other embodiments, there is provided a xerographic apparatus comprising: an imaging member, wherein an outermost layer of the imaging member comprises a structured organic film (SOF) comprising a plurality of segments and a plurality of linkers arranged as a covalent organic framework (COF), wherein the SOF comprises capping units and further wherein the capping units comprise hole transport molecules; a charging unit to impart an electrostatic charge on the imaging member; an exposure unit to create an electrostatic latent image on the imaging member; an image material delivery unit to create an image on the imaging member; a transfer unit to transfer the image from the imaging member; and an optional cleaning unit.

## BRIEF DESCRIPTION OF THE DRAWINGS

Other aspects of the present disclosure will become apparent as the following description proceeds and upon reference to the following figures which represent illustrative embodiments:

FIG. 1 illustrates the differences between typical SOF and a capped SOF. Left hand side: representation of a typical SOF network; right hand side: representation of capped SOF illustrating interruptions in the network and covalently linked capping group (circle).

FIG. 2 represents a simplified side view of an exemplary photoreceptor that incorporates a SOF of the present disclosure.

FIG. 3 represents a simplified side view of a second exemplary photoreceptor that incorporates a SOF of the present disclosure.

FIG. 4 represents a simplified side view of a third exemplary photoreceptor that incorporates a SOF of the present disclosure.

FIG. 5 represents a simplified schematic illustrating formation of a fluorinated SOF having hole transport molecule capping units according to the present disclosure.

Unless otherwise noted, the same reference numeral in different Figures refers to the same or similar feature.

#### DETAILED DESCRIPTION

“Structured organic film” (SOF) refers to a COF that is a film at a macroscopic level. The imaging members of the present disclosure comprise composite SOFs, which optionally may have a capping unit or group added into the SOF.

In this specification and the claims that follow, singular forms such as “a,” “an,” and “the” include plural forms unless the content clearly dictates otherwise.

The term “SOF” generally refers to a covalent organic framework (COO) that is a film at a macroscopic level. The phrase “macroscopic level” refers, for example, to the naked eye view of the present SOFs. Although COFs are a network at the “microscopic level” or “molecular level” (requiring use of powerful magnifying equipment or as assessed using scattering methods), the present SOF is fundamentally different at the “macroscopic level” because the film is for instance orders of magnitude larger in coverage than a microscopic level COF network. SOFs described herein have macroscopic morphologies much different than typical COFs previously synthesized.

Additionally, when a capping unit is introduced into the SOF, the SOF framework is locally ‘interrupted’ where the capping units are present. These SOF compositions are ‘covalently doped’ because a foreign molecule is bonded to the SOF framework when capping units are present. Capped SOF compositions may alter the properties of SOFs without changing constituent building blocks. For example, the mechanical and physical properties of the capped SOF where the SOF framework is interrupted may differ from that of an uncapped SOF.

The SOFs of the present disclosure are at the macroscopic level substantially pinhole-free SOFs or pinhole-free SOFs having continuous covalent organic frameworks that can extend over larger length scales such as for instance much greater than a millimeter to lengths such as a meter and, in theory, as much as hundreds of meters. It will also be appreciated that SOFs tend to have large aspect ratios where typically two dimensions of a SOF will be much larger than the third. SOFs have markedly fewer macroscopic edges and disconnected external surfaces than a collection of COF particles.

In embodiments, a “substantially pinhole-free SOF” or “pinhole-free SOF” may be formed from a reaction mixture deposited on the surface of an underlying substrate. The term “substantially pinhole-free SOF” refers, for example, to an SOF that may or may not be removed from the underlying substrate on which it was formed and contains substantially no pinholes, pores or gaps greater than the distance between the cores of two adjacent segments per square cm; such as, for example, less than 10 pinholes, pores or gaps greater than about 250 nanometers in diameter per cm<sup>2</sup>, or less than 5

pinholes, pores or gaps greater than about 100 nanometers in diameter per cm<sup>2</sup>. The term “pinhole-free SOF” refers, for example, to an SOF that may or may not be removed from the underlying substrate on which it was formed and contains no pinholes, pores or gaps greater than the distance between the cores of two adjacent segments per micron<sup>2</sup>, such as no pinholes, pores or gaps greater than about 500 Angstroms in diameter per micron<sup>2</sup>, or no pinholes, pores or gaps greater than about 250 Angstroms in diameter per micron<sup>2</sup>, or no pinholes, pores or gaps greater than about 100 Angstroms in diameter per micron<sup>2</sup>.

In embodiments, the SOF comprises at least one atom of an element that is not carbon, such at least one atom selected from the group consisting of hydrogen, oxygen, nitrogen, silicon, phosphorous, selenium, fluorine, boron, and sulfur. In further embodiments, the SOF is a boroxine, borazine-, borosilicate-, and boronate ester-free SOF.

The term “fluorinated SOF” refers, for example, to a SOF that contains fluorine atoms covalently bonded to one or more segment types or linker types of the SOF. The fluorinated SOFs of the present disclosure may further comprise fluorinated molecules that are not covalently bound to the framework of the SOF, but are randomly distributed in the fluorinated SOF composition (i.e., a composite fluorinated SOF). However, an SOF, which does not contain fluorine atoms covalently bonded to one or more segment types or linker types of the SOF, that merely includes fluorinated molecules that are not covalently bonded to one or more segments or linkers of the SOF is a composite SOF, not a fluorinated SOF.

Designing and tuning the fluorine content in the SOF compositions of the present disclosure is straightforward and neither requires synthesis of custom polymers, nor requires blending/dispersion procedures. Furthermore, the SOF compositions of the present disclosure may be SOF compositions in which the fluorine content is uniformly dispersed and patterned at the molecular level. Fluorine content in the SOFs of the present disclosure may be adjusted by changing the molecular building block used for SOF synthesis or by changing the amount of fluorine building block employed.

In embodiments, the fluorinated SOF may be made by the reaction of one or more suitable molecular building blocks, where at least one of the molecular building block segments comprises fluorine atoms.

#### Molecular Building Block

The SOFs of the present disclosure comprise molecular building blocks having a segment (S) and functional groups (Fg). Molecular building blocks require at least two functional groups (x≥2) and may comprise a single type or two or more types of functional groups. Functional groups are the reactive chemical moieties of molecular building blocks that participate in a chemical reaction to link together segments during the SOF forming process. A segment is the portion of the molecular building block that supports functional groups and comprises all atoms that are not associated with functional groups. Further, the composition of a molecular building block segment remains unchanged after SOF formation.

#### Functional Group

Functional groups are the reactive chemical moieties of molecular building blocks that may participate in a chemical reaction to link together segments during the SOF forming process. Functional groups may be composed of a single atom, or functional groups may be composed of more than one atom. The atomic compositions of functional groups are those compositions normally associated with reactive moieties in chemical compounds. Non-limiting examples of

functional groups include halogens, alcohols, ethers, ketones, carboxylic acids, esters, carbonates, amines, amides, imines, ureas, aldehydes, isocyanates, tosylates, alkenes, alkynes and the like.

Molecular building blocks contain a plurality of chemical moieties, but only a subset of these chemical moieties are intended to be functional groups during the SOF forming process. Whether or not a chemical moiety is considered a functional group depends on the reaction conditions selected for the SOF forming process. Functional groups (Fg) denote a chemical moiety that is a reactive moiety, that is, a functional group during the SOF forming process.

In the SOF forming process the composition of a functional group will be altered through the loss of atoms, the gain of atoms, or both the loss and the gain of atoms; or, the functional group may be lost altogether. In the SOF, atoms previously associated with functional groups become associated with linker groups, which are the chemical moieties that join together segments. Functional groups have characteristic chemistries and those of ordinary skill in the art can generally recognize in the present molecular building blocks the atom(s) that constitute functional group(s). It should be noted that an atom or grouping of atoms that are identified as part of the molecular building block functional group may be preserved in the linker group of the SOF. Linker groups are described below.

#### Capping Unit

Capping units of the present disclosure are molecules that 'interrupt' the regular network of covalently bonded building blocks normally present in an SOF. The differences between a SOF and a capped SOF are illustrated in FIG. 1. Capped SOF compositions are tunable materials whose properties can be varied through the type and amount of capping unit introduced. Capping units may comprise a single type or two or more types of functional groups and/or chemical moieties.

In embodiments, the capping units have a structure that is unrelated to the structure of any of the molecular building blocks that are added into the SOF formulation, which (after film formation) ultimately becomes the SOF.

In embodiments, the capping units have a structure that substantially corresponds to the structure of one of the molecular building blocks (such as the molecular building blocks for SOFs that are detailed in U.S. patent application Ser. Nos. 12/716,524; 12/716,449; 12/716,706; 12/716,324; 12/716,686; 12/716,571, and 12/815,688 which have been incorporated by reference) that is added to the SOF formulation, but one or more of the functional groups present on the building block is either missing or has been replaced with a different chemical moiety or functional group that will not participate in a chemical reaction (with the functional group(s) of the building blocks that are initially present) to link together segments during the SOF forming process.

In embodiments, the capping unit molecules may be 55 mono-functionalized. For example, in embodiments, the capping units may comprise only a single suitable or complementary functional group (as described above) that participates in a chemical reaction to link together segments during the SOF forming process and thus cannot bridge any further adjacent molecular building blocks (until a building block with a suitable or complementary functional group is added, such as when an additional SOF is formed on top of a capped SOF base layer and a multilayer SOF is formed).

When such capping units are introduced into the SOF coating formulation, upon curing, interruptions in the SOF framework are introduced. Interruptions in the SOF frame-

work are therefore sites where the single suitable or complementary functional group of the capping units have reacted with the molecular building block and locally terminate (or cap) the extension of the SOF framework and interrupt the regular network of covalently bonded building blocks normally present in an SOF. The type of capping unit (or structure or the capping unit) introduced into the SOF framework may be used to tune the properties of the SOF.

In embodiments, the capping unit molecules may comprise more than one chemical moiety or functional group. For example, the SOF coating formulation, which (after film formation), ultimately becomes bonded in the SOF may comprise a capping unit having at least two or more chemical moieties or functional groups, such as 2, 3, 4, 5, 6 or more chemical moieties or functional groups, where only one of the functional groups is a suitable or complementary functional group (as described above) that participates in a chemical reaction to link together segments during the SOF forming process. The various other chemical moieties or functional groups present on the molecular building block are chemical moieties or functional groups that are not suitable or complementary to participate in the specific chemical reaction to link together segments initially present during the SOF forming process and thus cannot bridge any further adjacent molecular building blocks. However, after the SOF is formed such chemical moieties and/or functional groups may be available for further reaction (similar to dangling functional groups, as discussed below) with additional components and thus allow for the further refining and tuning of the various properties of the formed SOF, or chemically attaching various other SOF layers in the formation of multilayer SOFs.

In embodiments, the molecular building blocks may have x functional groups (where x is three or more) and the capping unit molecules may comprise a capping unit molecule having x-1 functional groups that are suitable or complementary functional group (as described above) and participate in a chemical reaction to link together segments during the SOF forming process. For example, x would be 35 three for tris-(4-hydroxymethyl)triphenylamine (above), and x would be four for the building block illustrated below, N,N,N',N'-tetrakis-[(4-hydroxymethyl)phenyl]-biphenyl-4,4'-diamine:



A capping unit molecule having x-1 functional groups 60 that are suitable or complementary functional groups (as described above) and participate in a chemical reaction to link together segments during the SOF forming process would have 2 functional groups (for a molecular building block such as tris-(4-hydroxymethyl)triphenylamine), and 3 65 functional groups (for N,N,N',N'-tetrakis-[(4-hydroxymethyl)phenyl]-biphenyl-4,4'-diamine) that are suitable or complementary functional group (as described above) and

participate in a chemical reaction to link together segments during the SOF forming process. The other functional group present may be a chemical moiety or a functional group that is not suitable or complementary to participate in the specific chemical reaction to link together segments during the SOF fainting process and thus cannot bridge any further adjacent molecular building blocks. However, after the SOF is formed such functional groups may be available for further reaction with additional components and thus allowing for the further refining and tuning of the various properties of the formed SOF.

In embodiments, the capping unit may comprise a mixture of capping units, such as any combination of a first capping unit, a second capping unit, a third capping unit, a fourth capping unit, etc., where the structure of the capping unit varies. In embodiments, the structure of a capping unit or a combination of multiple capping units may be selected to either enhance or attenuate the chemical and physical properties of SOF; or the identity of the chemical moieties or functional group(s) on that are not suitable or complementary to participate in the chemical reaction to link together segments during the SOF forming process may be varied to form a mixture of capping units. Thus, the type of capping unit introduced into the SOF framework may be selected to introduce or tune a desired property of SOF.

In the present embodiments, the capping unit comprises one or more hole transport molecules or materials as discussed further below in regards to the charge transport layer. In particular, illustrative charge transport materials include for example a positive hole transporting material selected from compounds having in the main chain or the side chain a polycyclic aromatic ring such as anthracene, pyrene, phenanthrene, coronene, and the like, or a nitrogen-containing hetero ring such as indole, carbazole, oxazole, isoxazole, thiazole, imidazole, pyrazole, oxadiazole, mazoline, thiadiazole, triazole, and hydrazone compounds. Typical hole transport materials include electron donor materials, such as carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole); poly(vinylpyrene); poly(vinyltetraphene); poly(vinyltetracene) and poly(vinylperylene). Suitable electron transport materials include electron acceptors such as 2,4,7-trinitro-9-fluorenone; 4,5,7-tetrinitro-fluorenone; dinitroanthracene; dinitroacridene; tetracyanopyrene; dinitroanthraquinone; and butylcarbonylfluorenemalononitrile, see U.S. Pat. No. 4,921,769 the disclosure of which is incorporated herein by reference in its entirety. Other hole transporting materials include arylamines described in U.S. Pat. No. 4,265,990 the disclosure of which is incorporated herein by reference in its entirety, such as N,N'-diphenyl-N,N'-bis(alkylphenyl)-(1,1'-biphenyl)-4,4'-diamine wherein alkyl is selected from the group consisting of methyl, ethyl, propyl, butyl, hexyl, and the like. Other known charge transport layer molecules may be selected, reference for example U.S. Pat. Nos. 4,921,773 and 4,464,450 the disclosures of which are incorporated herein by reference in their entireties.

By incorporating excess hole transport molecules during the formation of the SOF, hole transport molecule capping units were able to bond to more than 50% of the available functional groups on the molecular building blocks (from which the linkers emerge). By incorporating these interruptions of capping units, the image quality of prints made with the imaging members unexpectedly improved. While the capping units reduced the amount of crosslinking in the SOF

network, the hole transport molecule presence was increased and prevented charge trapping during the xerographic cycling by improving charge mobility. It was shown that the increased charge mobility through the SOF layer reduced ghosting artifact.

#### Segment

A segment is the portion of the molecular building block that supports functional groups and comprises all atoms that are not associated with functional groups. Further, the composition of a molecular building block segment remains unchanged after SOF formation. In embodiments, the SOF may contain a first segment having a structure the same as or different from a second segment. In other embodiments, the structures of the first and/or second segments may be the same as or different from a third segment, forth segment, fifth segment, etc. A segment is also the portion of the molecular building block that can provide an inclined property. Inclined properties are described later in the embodiments.

In specific embodiments, the segment of the SOF comprises at least one atom of an element that is not carbon, such as at least one atom selected from the group consisting of hydrogen, oxygen, nitrogen, silicon, phosphorous, selenium, fluorine, boron, and sulfur.

A description of various exemplary molecular building blocks, linkers, SOF types, strategies to synthesize a specific SOF type with exemplary chemical structures, building blocks whose symmetrical elements are outlined, and classes of exemplary molecular entities and examples of members of each class that may serve as molecular building blocks for SOFs are detailed in U.S. patent application Ser. Nos. 12/716,524; 12/716,449; 12/716,706; 12/716,324; 12/716,686; and 12/716,571 entitled "Structured Organic Films," "Structured Organic Films Having an Added Functionality," "Mixed Solvent Process for Preparing Structured Organic Films," "Composite Structured Organic Films," "Process For Preparing Structured Organic Films (SOFs) Via a Pre-SOF," "Electronic Devices Comprising Structured Organic Films," the disclosures of which are totally incorporated herein by reference in their entireties.

#### Linker

A linker is a chemical moiety that emerges in a SOF upon chemical reaction between functional groups present on the molecular building blocks and/or capping unit.

A linker may comprise a covalent bond, a single atom, or a group of covalently bonded atoms. The former is defined as a covalent bond linker and may be, for example, a single covalent bond or a double covalent bond and emerges when functional groups on all partnered building blocks are lost entirely. The latter linker type is defined as a chemical moiety linker and may comprise one or more atoms bonded together by single covalent bonds, double covalent bonds, or combinations of the two. Atoms contained in linking groups originate from atoms present in functional groups on molecular building blocks prior to the SOF forming process. Chemical moiety linkers may be well-known chemical groups such as for example, esters, ketones, amides, imines, ethers, urethanes, carbonates, and the like, or derivatives thereof.

For example, when two hydroxyl (—OH) functional groups are used to connect segments in a SOF via an oxygen atom, the linker would be the oxygen atom, which may also be described as an ether linker. In embodiments, the SOF may contain a first linker having a structure the same as or different from a second linker. In other embodiments, the structures of the first and/or second linkers may be the same as or different from a third linker, etc.

A capping unit may be bonded in the SOF in any desired amount as long as the general SOF framework is sufficiently maintained. For example, in embodiments, a capping unit may be bonded to at least 01% of all linkers, but not more than about 40% of all linkers present in an SOF, such as from about 0.5% to about 30%, or from about 2% to about 20%. In the event capping units bond to more than 50% of the available functional groups on the molecular building blocks (from which the linkers emerge), oligomers, linear polymers, and molecular building blocks that are fully capped with capping units may predominately form instead of a SOF.

In specific embodiments, the linker comprises at least one atom of an element that is not carbon, such at least one atom selected from the group consisting of hydrogen, oxygen, nitrogen, silicon, phosphorous, selenium, fluorine, boron, and sulfur.

In embodiments, a SOF contains segments, which are not located at the edges of the SOF, that are connected by linkers to at least three other segments and/or capping groups. For example, in embodiments the SOF comprises at least one symmetrical building block selected from the group consisting of ideal triangular building blocks, distorted triangular building blocks, ideal tetrahedral building blocks, distorted tetrahedral building blocks, ideal square building blocks, and distorted square building blocks. In embodiments, Type 2 and 3 SOF contains at least one segment type, which are not located at the edges of the SOF, that are connected by linkers to at least three other segments and/or capping groups. For example, in embodiments the SOF comprises at least one symmetrical building block selected from the group consisting of ideal triangular building blocks, distorted triangular building blocks, ideal tetrahedral building blocks, distorted tetrahedral building blocks, ideal square building blocks, and distorted square building blocks.

In embodiments, the SOF comprises a plurality of segments, where all segments have an identical structure, and a plurality of linkers, which may or may not have an identical structure, wherein the segments that are not at the edges of the SOF are connected by linkers to at least three other segments and/or capping groups. In embodiments, the SOF comprises a plurality of segments where the plurality of segments comprises at least a first and a second segment that are different in structure, and the first segment is connected by linkers to at least three other segments and/or capping groups when it is not at the edge of the SOF.

In embodiments, the SOF comprises a plurality of linkers including at least a first and a second linker that are different in structure, and the plurality of segments either comprises at least a first and a second segment that are different in structure, where the first segment, when not at the edge of the SOF, is connected to at least three other segments and/or capping groups, wherein at least one of the connections is via the first linker, and at least one of the connections is via the second linker; or comprises segments that all have an identical structure, and the segments that are not at the edges of the SOF are connected by linkers to at least three other segments and/or capping groups, wherein at least one of the connections is via the first linker, and at least one of the connections is via the second linker.

#### Metrical Parameters of SOFs

SOFs have any suitable aspect ratio. In embodiments, SOFs have aspect ratios for instance greater than about 30:1 or greater than about 50:1, or greater than about 70:1, or greater than about 100:1, such as about 1000:1. The aspect ratio of a SOF is defined as the ratio of its average width or diameter (that is, the dimension next largest to its thickness)

to its average thickness (that is, its shortest dimension). The term ‘aspect ratio,’ as used here, is not bound by theory. The longest dimension of a SOF is its length and it is not considered in the calculation of SOF aspect ratio.

Generally, SOFs have widths and lengths, or diameters greater than about 500 micrometers, such as about 10 mm, or 30 mm. The SOFs have the following illustrative thicknesses: about 10 Angstroms to about 250 Angstroms, such as about 20 Angstroms to about 200 Angstroms, for a mono-segment thick layer and about 20 nm to about 5 mm, about 50 nm to about 10 mm for a multi-segment thick layer.

SOF dimensions may be measured using a variety of tools and methods. For a dimension about 1 micrometer or less, scanning electron microscopy is the preferred method. For a dimension about 1 micrometer or greater, a micrometer (or ruler) is the preferred method.

#### Multilayer SOFs

A SOF may comprise a single layer or a plurality of layers (that is, two, three or more layers). SOFs that are comprised of a plurality of layers may be physically joined (e.g., dipole and hydrogen bond) or chemically joined. Physically attached layers are characterized by weaker interlayer interactions or adhesion; therefore physically attached layers may be susceptible to delamination from each other. Chemically attached layers are expected to have chemical bonds (e.g., covalent or ionic bonds) or have numerous physical or intermolecular (supramolecular) entanglements that strongly link adjacent layers.

Therefore, delamination of chemically attached layers is much more difficult. Chemical attachments between layers may be detected using spectroscopic methods such as focusing infrared or Raman spectroscopy, or with other methods having spatial resolution that can detect chemical species precisely at interfaces. In cases where chemical attachments between layers are different chemical species than those within the layers themselves it is possible to detect these attachments with sensitive bulk analyses such as solid-state nuclear magnetic resonance spectroscopy or by using other bulk analytical methods.

In the embodiments, the SOF may be a single layer (mono-segment thick or multi-segment thick) or multiple layers (each layer being mono-segment thick or multi-segment thick). “Thickness” refers, for example, to the smallest dimension of the film. As discussed above, in a SOF, segments are molecular units that are covalently bonded through linkers to generate the molecular framework of the film. The thickness of the film may also be defined in terms of the number of segments that is counted along that axis of the film when viewing the cross-section of the film. “monolayer” SOF is the simplest case and refers, for example, to where a film is one segment thick. A SOF where two or more segments exist along this axis is referred to as a “multi-segment” thick SOF.

An exemplary method for preparing physically attached multilayer SOFs includes: (1) forming a base SOF layer that may be cured by a first curing cycle, and (2) forming upon the base layer a second reactive wet layer followed by a second curing cycle and, if desired, repeating the second step to form a third layer, a forth layer and so on. The physically stacked multilayer SOFs may have thicknesses greater than about 20 Angstroms such as, for example, the following illustrative thicknesses: about 20 Angstroms to about 10 cm, such as about 1 nm to about 10 mm, or about 0.1 mm Angstroms to about 5 mm. In principle there is no limit with this process to the number of layers that may be physically stacked.

## 11

In embodiments, a multilayer SOF is formed by a method for preparing chemically attached multilayer SOB by: (1) forming a base SOF layer having functional groups present on the surface (or dangling functional groups) from a first reactive wet layer, and (2) forming upon the base layer a second SOF layer from a second reactive wet layer that comprises molecular building blocks with functional groups capable of reacting with the dangling functional groups on the surface of the base SOF layer, in further embodiments, a capped SOF may serve as the base layer in which the functional groups present that were not suitable or complementary to participate in the specific chemical reaction to link together segments during the base layer SOF forming process may be available for reacting with the molecular building blocks of the second layer to form a chemically bonded multilayer SOF. If desired, the formulation used to form the second SOF layer should comprise molecular building blocks with functional groups capable of reacting with the functional groups from the base layer as well as additional functional groups that will allow for a third layer to be chemically attached to the second layer. The chemically stacked multilayer SOFs may have thicknesses greater than about 20 Angstroms such as, for example, the following illustrative thicknesses: about 20 Angstroms to about 10 cm, such as about 1 nm to about 10 mm, or about 0.1 mm Angstroms to about 5 mm. In principle there is no limit with this process to the number of layers that may be chemically stacked.

In embodiments, the method for preparing chemically attached multilayer SOFs comprises promoting chemical attachment of a second SOF onto an existing SOF (base layer) by using a small excess of one molecular building block (when more than one molecular building block is present) during the process used to form the SOF (base layer) whereby the functional groups present on this molecular building block will be present on the base layer surface. The surface of base layer may be treated with an agent to enhance the reactivity of the functional groups or to create an increased number of functional groups.

In an embodiment the dangling functional groups or chemical moieties present on the surface of an SOF or capped SOF may be altered to increase the propensity for covalent attachment (or, alternatively, to disfavor covalent attachment) of particular classes of molecules or individual molecules, such as SOFs, to a base layer or any additional substrate or SOF layer. For example, the surface of a base layer, such as an SOF layer, which may contain reactive dangling functional groups, may be rendered pacified through surface treatment with a capping chemical group. For example, a SOF layer having dangling hydroxyl alcohol groups may be pacified by treatment with trimethylsilylchloride thereby capping hydroxyl groups as stable trimethylsilyl ethers. Alternatively, the surface of base layer may be treated with a non-chemically bonding agent, such as a wax, to block reaction with dangling functional groups from subsequent layers.

#### Molecular Building Block Symmetry

Molecular building block symmetry relates to the positioning of functional groups (Fgs) around the periphery of the molecular building block segments. Without being bound by chemical or mathematical theory, a symmetric molecular building block is one where positioning of Fgs may be associated with the ends of a rod, vertexes of a regular geometric shape, or the vertexes of a distorted rod or distorted geometric shape. For example, the most symmetric

## 12

option for molecular building blocks containing four Fgs are those whose Fgs overlay with the corners of a square or the apexes of a tetrahedron.

Use of symmetrical building blocks is practiced in embodiments of the present disclosure for two reasons: (1) the patterning of molecular building blocks may be better anticipated because the linking of regular shapes is a better understood process in reticular chemistry, and (2) the complete reaction between molecular building blocks is facilitated because for less symmetric building blocks errant conformations/orientations may be adopted which can possibly initiate numerous linking defects within SOFs.

In embodiments, a Type 1 SOF contains segments, which are not located at the edges of the SOF, that are connected by linkers to at least three other segments. For example, in embodiments the SOF comprises at least one symmetrical building block selected from the group consisting of ideal triangular building blocks, distorted triangular building blocks, ideal tetrahedral building blocks, distorted tetrahedral building blocks, ideal square building blocks, and distorted square building blocks. In embodiments, Type 2 and 3 SOF contains at least one segment type, which are not located at the edges of the SOF, that are connected by linkers to at least three other segments. For example, in embodiments the SOF comprises at least one symmetrical building block selected from the group consisting of ideal triangular building blocks, distorted triangular building blocks, ideal tetrahedral building blocks, distorted tetrahedral building blocks, ideal square building blocks, and distorted square building blocks.

#### Practice of Linking Chemistry

In embodiments linking chemistry may occur wherein the reaction between functional groups produces a volatile byproduct that may be largely evaporated or expunged from the SOF during or after the film forming process or wherein no byproduct is formed. Linking chemistry may be selected to achieve a SOF for applications where the presence of linking chemistry byproducts is not desired. Linking chemistry reactions may include, for example, condensation, addition elimination, and addition reactions, such as, for example, those that produce esters, imines, ethers, carbonates, urethanes, amides, acetals, and silyl ethers.

In embodiments the linking chemistry via a reaction between function groups producing a non-volatile byproduct that largely remains incorporated within the SOF after the film forming process. Linking chemistry in embodiments may be selected to achieve a SOF for applications where the presence of linking chemistry byproducts does not impact the properties or for applications where the presence of linking chemistry byproducts may alter the properties of a SOF (such as, for example, the electroactive, hydrophobic or hydrophilic nature of the SOF). Linking chemistry reactions may include, for example, substitution, metathesis, and metal catalyzed coupling reactions, such as those that produce carbon-carbon bonds.

For all linking chemistry the ability to control the rate and extent of reaction between building blocks via the chemistry between building block functional groups is an important aspect of the present disclosure. Reasons for controlling the rate and extent of reaction may include adapting the film forming process for different coating methods and tuning the microscopic arrangement of building blocks to achieve a periodic SOF, as defined in earlier embodiments.

#### Innate Properties of COFs

COFs have innate properties such as high thermal stability (typically higher than 400° C. under atmospheric conditions); poor solubility in organic solvents (chemical stabil-

13

ity), and porosity (capable of reversible guest uptake). In embodiments, SOFs may also possess these innate properties.

#### Added Functionality of SOFs

Added functionality denotes a property that is not inherent to conventional COFs and may occur by the selection of molecular building blocks wherein the molecular compositions provide the added functionality in the resultant SOF. Added functionality may arise upon assembly of molecular building blocks and/or capping units having an “inclined property” for that added functionality. Added functionality may also arise upon assembly of molecular building blocks having no “inclined property” for that added functionality but the resulting SOF has the added functionality as a consequence of linking segments (S) and linkers into a SOF. In embodiments, added functionality may also arise upon the addition and assembly of molecular building blocks and capping units having no “inclined property” for that added functionality but the resulting SOF has the added functionality as a consequence of linking segments, linkers, and capping units into a SOF. Furthermore, emergence of added functionality may arise from the combined effect of using molecular building blocks bearing an “inclined property” for that added functionality whose inclined property is modified or enhanced upon linking together the segments and linkers into a SOF.

#### An Inclined Property of a Molecular Building Block

The term “inclined property” of a molecular building block refers, for example, to a property known to exist for certain molecular compositions or a property that is reasonably identifiable by a person skilled in art upon inspection of the molecular composition of a segment. As used herein, the terms “inclined property” and “added functionality” refer to the same general property (e.g., hydrophobic, electroactive, etc.) but “inclined property” is used in the context of the molecular building block and “added functionality” is used in the context of the SOF.

The hydrophobic (superhydrophobic), hydrophilic, lipophobic (superlipophobic), lipophilic, photochromic and/or electroactive (conductor, semiconductor, charge transport material) nature of an SOF are some examples of the properties that may represent an “added functionality” of an SOF. These and other added functionalities may arise from the inclined properties of the molecular building blocks or may arise from building blocks that do not have the respective added functionality that is observed in the SOF.

The term hydrophobic (superhydrophobic) refers, for example, to the property of repelling water, or other polar species such as methanol, it also means an inability to absorb water and/or to swell as a result. Furthermore, hydrophobic implies an inability to form strong hydrogen bonds to water or other hydrogen bonding species. Hydrophobic materials are typically characterized by having water contact angles greater than 90° and superhydrophobic materials have water contact angles greater than 150° as measured using a contact angle goniometer or related device.

The term hydrophilic refers, for example, to the property of attracting, adsorbing, or absorbing water or other polar species, or a surface that is easily wetted by such species. Hydrophilic materials are typically characterized by having less than 20° water contact angle as measured using a contact angle goniometer or related device. Hydrophilicity may also be characterized by swelling of a material by water or other polar species, or a material that can diffuse or transport water, or other polar species, through itself, Hydro-

14

philicity, is further characterized by being able to form strong or numerous hydrogen bonds to water or other hydrogen bonding species.

The term lipophobic (oleophobic) refers, for example, to the property of repelling oil or other non-polar species such as alkanes, fats, and waxes. Lipophobic materials are typically characterized by having oil contact angles greater than 90° as measured using a contact angle goniometer or related device.

The term lipophilic (oleophilic) refers, for example, to the property attracting oil or other non-polar species such as alkanes, fats, and waxes or a surface that is easily wetted by such species. Lipophilic materials are typically characterized by having a low to nil oil contact angle as measured using, for example, a contact angle goniometer. Lipophilicity can also be characterized by swelling of a material by hexane or other non-polar liquids.

The term photochromic refers, for example, to the ability to demonstrate reversible color changes when exposed to electromagnetic radiation. SOF compositions containing photochromic molecules may be prepared and demonstrate reversible color changes when exposed to electromagnetic radiation. These SOFs may have the added functionality of photochromism. The robustness of photochromic SOFs may enable their use in many applications, such as photochromic SOFs for erasable paper, and light responsive films for window tinting/shading and eye wear. SOF compositions may contain any suitable photochromic molecule, such as a difunctional photochromic molecules as SOF molecular building blocks (chemically bound into SOF structure), a monofunctional photochromic molecules as SOF capping units (chemically bound into SOF structure, or unfunctionalized photochromic molecules in an SOF composite (not chemically bound into SOF structure). Photochromic SOFs may change color upon exposure to selected wavelengths of light and the color change may be reversible.

SOF compositions containing photochromic molecules that chemically bond to the SOF structure are exceptionally chemically and mechanically robust photochromic materials. Such photochromic SOF materials demonstrate many superior properties, such as high number of reversible color change processes, to available polymeric alternatives.

The term electroactive refers, for example, to the property to transport electrical charge (electrons and/or holes). Electroactive materials include conductors, semiconductors, and charge transport materials. Conductors are defined as materials that readily transport electrical charge in the presence of a potential difference. Semiconductors are defined as materials do not inherently conduct charge but may become conductive in the presence of a potential difference and an applied stimuli, such as, for example, an electric field, electromagnetic radiation, heat, and the like. Charge transport materials are defined as materials that can transport charge when charge is injected from another material such as, for example, a dye, pigment, or metal in the presence of a potential difference.

Conductors may be further defined as materials that give a signal using a potentiometer from about 0.1 to about 10<sup>7</sup> S/cm.

Semiconductors may be further defined as materials that give a signal using a potentiometer from about 10<sup>-6</sup> to about 10<sup>4</sup> S/cm in the presence of applied stimuli such as, for example an electric field, electromagnetic radiation, heat, and the like. Alternatively, semiconductors may be defined as materials having electron and/or hole mobility measured using time-of-flight techniques in the range of 10<sup>-10</sup> to about

15

$10^6 \text{ cm}^2 \text{V}^{-1} \text{s}^{-1}$  when exposed to applied stimuli such as, for example an electric field, electromagnetic radiation, heat, and the like.

Charge transport materials may be further defined as materials that have electron and/or hole mobility measured using time-of-flight techniques in the range of  $10^{-10}$  to about  $10^6 \text{ cm}^2 \text{V}^{-1} \text{s}^{-1}$ . It should be noted that under some circumstances charge transport materials may be also classified as semiconductors.

SOFs with hydrophobic added functionality may be prepared by using molecular building blocks with inclined hydrophobic properties and/or have a rough, textured, or porous surface on the sub-micron to micron scale. A paper describing materials having a rough, textured, or porous surface on the sub-micron to micron scale being hydrophobic was authored by Cassie and Baxter (Cassie, A. B. D.; Baxter, S. Trans. Faraday Soc., 1944, 40, 546).

Molecular building blocks comprising or bearing highly-fluorinated segments have inclined hydrophobic properties and may lead to SOFs with hydrophobic added functionality. Highly-fluorinated segments are defined as the number of fluorine atoms present on the segment(s) divided by the number of hydrogen atoms present on the segment(s) being greater than one. Fluorinated segments, which are not highly-fluorinated segments may also lead to SOFs with hydrophobic added functionality.

The above-mentioned fluorinated segments may include, for example, tetrafluorohydroquinone, perfluoroadipic acid hydrate, 4,4'-(hexafluoroisopropylidene)diphthalic anhydride, 4,4'-(hexafluoroisopropylidene)diphenol, and the like.

SOFs having a rough, textured, or porous surface on the sub-micron to micron scale may also be hydrophobic. The rough, textured, or porous SOF surface can result from dangling functional groups present on the film surface or from the structure of the SOF. The type of pattern and degree of patterning depends on the geometry of the molecular building blocks and the linking chemistry efficiency. The feature size that leads to surface roughness or texture is from about 100 nm to about such as from about 500 nm to about 5  $\mu\text{m}$ .

SOFs with hydrophilic added functionality may be prepared by using molecular building blocks with inclined hydrophilic properties and/or comprising polar linking groups.

Molecular building blocks comprising segments bearing polar substituents have inclined hydrophilic properties and may lead to SOFs with hydrophilic added functionality. The term polar substituents refers, for example, to substituents that can form hydrogen bonds with water and include, for example, hydroxyl, amino, ammonium, and carbonyl (such as ketone, carboxylic acid, ester, amide, carbonate, urea).

SOFs with electroactive added functionality may be prepared by using molecular building blocks with inclined electroactive properties and/or be electroactive resulting from the assembly of conjugated segments and linkers. The following sections describe molecular building blocks with inclined hole transport properties, inclined electron transport properties, and inclined semiconductor properties.

SOB with hole transport added functionality may be obtained by selecting segment cores such as, for example, triarylamines, hydrazones (U.S. Pat. No. 7,202,002 B2 to Tokarski et al.), and enamines (U.S. Pat. No. 7,416,824 B2 to Kondoh et al.) with the following general structures:

16



The segment core comprising a triarylamine being represented by the following general formula:



wherein Ar<sup>1</sup>, Ar<sup>2</sup>, Ar<sup>3</sup>, Ar<sup>4</sup> and Ar<sup>5</sup> each independently represents a substituted or unsubstituted aryl group, or Ar<sup>5</sup> independently represents a substituted or unsubstituted arylene group, and k represents 0 or 1, wherein at least two of Ar<sup>1</sup>, Ar<sup>2</sup>, Ar<sup>3</sup>, Ar<sup>4</sup> and Ar<sup>5</sup> comprises a Fg (previously defined). Ar<sup>5</sup> may be further defined as, for example, a substitute phenyl ring; substituted/unsubstituted phenylene, substituted/unsubstituted monovalently linked aromatic rings such as biphenyl, terphenyl, and the like, or substituted/unsubstituted fused aromatic rings such as naphthyl, anthranyl, phenanthryl, and the like.

Segment cores comprising arylamines with hole transport added functionality include, for example, aryl amines such as triphenylamine, N,N,N',N'-tetraphenyl-(1,1'-biphenyl)-4,4'-diamine, N,N'-diphenyl-N,N'-bis(3-methylphenyl)-(1,1'-biphenyl)-4,4'-diamine, N,N'-bis(4-butylphenyl)-N,N'-diphenyl-[p-terphenyl]-4,4"-diamine; hydrazones such as N-phenyl-N-methyl-3-(9-ethyl)carbazyl hydrazone and 4-diethyl amino benzaldehyde-1,2-diphenyl hydrazone and oxadiazoles such as 2,5-bis(4-N,N'-diethylaminophenyl)-1,2,4-oxadiazole, stilbenes, and the like.

Molecular building blocks comprising triarylamine core segments with inclined hole transport properties may be derived from the list of chemical structures including, for example, those listed below:



**17**  
-continued



**18**  
-continued



The segment core comprising a hydrazone being represented by the following general formula:

60



65

19

wherein  $\text{Ar}^1$ ,  $\text{Ar}^2$ , and  $\text{Ar}^3$  each independently represents an aryl group optionally containing one or more substituents, and R represents a hydrogen atom, an aryl group, or an alkyl group optionally containing a substituent; wherein at least two of  $\text{Ar}^1$ ,  $\text{Ar}^2$ , and  $\text{Ar}^3$  comprises a  $\text{Fg}$  (previously defined); and a related oxadiazole being represented by the following general formula:



10

wherein Ar and  $\text{Ar}^1$  each independently represent an aryl group that comprises a  $\text{Fg}$  (previously defined).

Molecular building blocks comprising hydrazone and oxadiazole core segments with inclined hole transport properties may be derived from the list of chemical structures including, for example, those listed below:



25



40



55

20

-continued



The segment core comprising an enamine being represented by the following general formula:



60

wherein  $\text{Ar}^1$ ,  $\text{Ar}^2$ ,  $\text{Ar}^3$ , and  $\text{Ar}^4$  each independently represents an aryl group that optionally contains one or more substituents or a heterocyclic group that optionally contains one or more substituents, and R represents a hydrogen atom,

**21**

an aryl group, or an alkyl group optionally containing a substituent; wherein at least two of  $\text{Ar}^1$ ,  $\text{Ar}^2$ ,  $\text{Ar}^3$ , and  $\text{Ar}^4$  comprises a  $\text{Fg}$  (previously defined).

Molecular building blocks comprising enamine core segments with inclined hole transport properties may be derived from the list of chemical structures including, for example, those listed below:



10



20



30



40



50



60

65

**22**  
-continued



15



25



40



55

23

-continued



SOFs with electron transport added functionality may be obtained by selecting segment cores comprising, for example, nitrofluorenones, 9-fluorenylidene malonitriles, diphenoquinones, and naphthalenetetracarboxylic diimides with the following general structures:



It should be noted that the carbonyl groups of diphenylquinones could also act as Fgs in the SOF forming process.

SOFs with semiconductor added functionality may be obtained by selecting segment cores such as, for example, acenes, thiophenes/oligothiophenes/fused thiophenes, perylene bisimides, or tetrathiofulvalenes, and derivatives thereof with the following general structures:

24



The SOF may be a p-type, semiconductor, n-type semiconductor or ambipolar semiconductor. The SOF semiconductor type depends on the nature of the molecular building blocks. Molecular building blocks that possess an electron donating property such as alkyl, alkoxy, aryl, and amino groups, when present in the SOF, may render the SOF a p-type semiconductor. Alternatively, molecular building blocks that are electron withdrawing such as cyano, nitro, fluoro, fluorinated alkyl, and fluorinated aryl groups may render the SOF into the n-type semiconductor.

Molecular building blocks comprising acene core segments with inclined semiconductor properties may be derived from the list of chemical structures including, for example, those listed below:



25

-continued



26

-continued



Molecular building blocks comprising thiophene/oliphthiophene/fused thiophene core segments with inclined semiconductor properties may be derived from the list of chemical structures including, for example, those listed below:



Examples of molecular building blocks comprising perylene bisimide core segments with inclined semiconductor properties may be derived from the chemical structure below:



Molecular building blocks comprising tetrathiofulvalene core segments with inclined semiconductor properties may be derived from the list of chemical structures including, for example, those listed below:



-continued



wherein Ar each independently represents an aryl group that optionally contains one or more substituents or a heterocyclic group that optionally contains one or more substituents. Similarly, the electroactivity of SOFs prepared by these molecular building blocks will depend on the nature of the segments, nature of the linkers, and how the segments are orientated within the SOF. Linkers that favor preferred orientations of the segment moieties in the SOF are expected to lead to higher electroactivity.

Process for Preparing a Capped Structured Organic Film (SOF)

The process for making capped SOFs (which may be referred to as an "SOF" below) typically comprises a similar number of activities or steps (set forth below) that are used to make a non-capped SOF. The capping unit may be added during either step a, b or c, depending the desired distribution of the capping unit in the resulting SOF. For example, if it is desired that the capping unit distribution is substantially uniform over the resulting SOF, the capping unit may be added during step a. Alternatively, if, for example, a more heterogeneous distribution of the capping unit is desired, adding the capping unit (such as by spraying it on the film formed during step b or during the promotion step of step c) may occur during steps b and c.

The process for making SOFs typically comprises a number of activities or steps (set forth below) that may be performed in any suitable sequence or where two or more activities are performed simultaneously or in close proximity in time:

A process for preparing a structured organic film comprising:

- preparing a liquid-containing reaction mixture comprising a plurality of molecular building blocks each comprising a segment and a number of functional groups;
- depositing the reaction mixture as a wet film;
- promoting a change of the wet film including the molecular building blocks to a dry film comprising the

SOF comprising a plurality of the segments and a plurality of linkers arranged as a covalent organic framework, wherein at a macroscopic level the covalent organic framework is a film;

- optionally removing the SOF from the coating substrate to obtain a free-standing SOF;
- optionally processing the free-standing SOF into a roll;
- optionally cutting and seaming the SOF into a belt; and
- optionally performing the above SOF formation process(es) upon an SOF (which was prepared by the above SOF formation process(es)) as a substrate for subsequent SOF formation process(es).

The above activities or steps may be conducted at atmospheric, super atmospheric, or subatmospheric pressure. The term "atmospheric pressure" as used herein refers to a pressure of about 760 torr. The term "super atmospheric" refers to pressures greater than atmospheric pressure, but less than 20 atm. The term "subatmospheric pressure" refers to pressures less than atmospheric pressure. In an embodiment, the activities or steps may be conducted at or near atmospheric pressure. Generally, pressures of from about 0.1 atm to about 2 atm, such as from about 0.5 atm to about 1.5 atm, or 0.8 atm to about 1.2 atm may be conveniently employed.

25 Process Action A: Preparation of the Liquid-Containing Reaction Mixture

The reaction mixture comprises a plurality of molecular building blocks that are dissolved, suspended, or mixed in a liquid. The plurality of molecular building blocks may be of one type or two or more types. When one or more of the molecular building blocks is a liquid, the use of an additional liquid is optional. Catalysts may optionally be added to the reaction mixture to enable SOF formation or modify the kinetics of SOF formation during Action C described above. Additives or secondary components may optionally be added to the reaction mixture to alter the physical properties of the resulting SOF.

The reaction mixture components (molecular building blocks, optionally a capping unit, liquid, optionally catalysts, and optionally additives) are combined in a vessel. The order of addition of the reaction mixture components may vary; however, typically the catalyst is added last. In particular embodiments, the molecular building blocks are heated in the liquid in the absence of the catalyst to aid the dissolution of the molecular building blocks. The reaction mixture may also be mixed, stirred, milled, or the like, to ensure even distribution of the formulation components prior to depositing the reaction mixture as a wet film.

In embodiments, the reaction mixture may be heated prior to being deposited as a wet film. This may aid the dissolution of one or more of the molecular building blocks and/or increase the viscosity of the reaction mixture by the partial reaction of the reaction mixture prior to depositing the wet layer. This approach may be used to increase the loading of the molecular building blocks in the reaction mixture.

In particular embodiments, the reaction mixture needs to have a viscosity that will support the deposited wet layer. Reaction mixture viscosities range from about 10 to about 50,000 cps, such as from about 25 to about 25,000 cps or from about 50 to about 1000 cps.

The molecular building block and capping unit loading or "loading" in the reaction mixture is defined as the total weight of the molecular building blocks and optionally the capping units and catalysts divided by the total weight of the reaction mixture. Building block loadings may range from about 3 to 100%, such as from about 5 to about 50%, or from about 15 to about 40%. In the case where a liquid molecular

building block is used as the only liquid component of the reaction mixture (i.e. no additional liquid is used), the building block loading would be about 100%. The capping unit loading may be chosen, so as to achieve the desired loading of the capping group. For example, depending on when the capping unit is to be added to the reaction mixture, capping unit loadings may range, by weight, from about 3 to 80%, such as from about 5 to about 50%, or from about 15 to about 40% by weight.

In embodiments, the theoretical upper limit for capping unit molecular building loading in the reaction mixture (liquid SOF formulation) is the molar amount of capping units that reduces the number of available linking groups to 2 per molecular building block in the liquid SOF formulation. In such a loading, substantial SOF formation may be effectively inhibited by exhausting (by reaction with the respective capping group) the number of available linkable functional groups per molecular building block. For example, in such a situation (where the capping unit loading is in an amount sufficient to ensure that the molar excess of available linking groups is less than 2 per molecular building block in the liquid SOF formulation), oligomers, linear polymers, and molecular building blocks that are fully capped with capping units may predominately form instead of an SOF.

In embodiments, the capping unit building block loading of the SOF liquid formulation may be used to adjust or modulate the concentration of capping units that are ultimately incorporated in the dry SOF. Thus, the wear rate of the dry SOF of the imaging member or a particular layer of the imaging member may be adjusted or modulated by selecting a predetermined capping unit building block loading of the SOF liquid formulation. In further embodiments, the predetermined capping unit may be pre-installed on a building block prior to the SOF forming process, or in specific embodiments, may be building block Fg that remains unreacted in the SOF by using a sub-stoichiometric amount of complementary building block. In embodiments, an effective capping unit and/or effective capping unit concentration in the dry SOF may be selected to either decrease the wear rate of the imaging member or increase the wear rate of the imaging member. In embodiments, the wear rate of the imaging member may be decreased by at least about 2% per 1000 cycles, such as by at least about 5% per 100 cycles, or at least 10% per 1000 cycles relative to a non-capped SOF comprising the same segment(s) and linker(s).

Liquids used in the reaction mixture may be pure liquids, such as solvents, and/or solvent mixtures. Liquids are used to dissolve or suspend the molecular building blocks and catalyst/modifiers in the reaction mixture. Liquid selection is generally based on balancing the solubility/dispersion of the molecular building blocks and a particular building block loading, the viscosity of the reaction mixture, and the boiling point of the liquid, which impacts the promotion of the wet layer to the dry SOF. Suitable liquids may have boiling points from about 30 to about 300° C., such as from about 65° C. to about 250° C., or from about 100° C. to about 180° C.

Liquids can include molecule classes such as alkanes (hexane, heptane, octane, nonane, decane, cyclohexane, cycloheptane, cyclooctane, decalin); mixed alkanes (hexanes, heptanes); branched alkanes (isooctane); aromatic compounds (toluene, o-, m-, p-xylene, mesitylene, nitrobenzene, benzonitrile, butylbenzene, aniline); ethers (benzyl ethyl ether, butyl ether, isoamyl ether, propyl ether); cyclic ethers (tetrahydrofuran, dioxane); esters (ethyl acetate, butyl acetate, butyl butyrate, ethoxyethyl acetate, ethyl propi-

onate, phenyl acetate, methyl benzoate); ketones (acetone, methyl ethyl ketone, methyl isobutylketone, diethyl ketone, chloroacetone, 2-heptanone), cyclic ketones (cyclopentanone, cyclohexanone), amines (1°, 2°, or 3° amines such as butylamine, diisopropylamine, triethylamine, diisopropylethylamine; pyridine); amides (dimethylformamide, N-methylpyrrolidinone, N,N-dimethylformamide); alcohols (methanol, ethanol, n-, i-propanol, n-, t-butanol, 1-methoxy-2-propanol hexanol, cyclohexanol, 3-pentanol, benzyl alcohol); nitriles (acetonitrile, benzonitrile, butyronitrile), halogenated aromatics (chlorobenzene, dichlorobenzene, hexafluorobenzene), halogenated alkanes (dichloromethane, chloroform, dichloroethylene, tetrachloroethane); and water.

Mixed liquids comprising a first solvent, second solvent, 15 third solvent, and so forth may also be used in the reaction mixture. Two or more liquids may be used to aid the dissolution/dispersion of the molecular building blocks; and/or increase the molecular building block loading; and/or allow a stable wet film to be deposited by aiding the wetting of the substrate and deposition instrument; and/or modulate the promotion of the wet layer to the dry SOF. In embodiments, the second solvent is a solvent whose boiling point or vapor-pressure curve or affinity for the molecular building blocks differs from that of the first solvent. In embodiments, 20 a first solvent has a boiling point higher than that of the second solvent. In embodiments, the second solvent has a boiling point equal to or less than about 100° C., such as in the range of from about 30° C. to about 100° C., or in the range of from about 40° C. to about 90° C., or about 50° C. to about 80° C.

In embodiments, the first solvent, or higher boiling point solvent, has a boiling point equal to or greater than about 65° C., such as in the range of from about 80° C. to about 300° C., or in the range of from about 100° C. to about 250° C., or about 100° C. to about 180° C. The higher boiling point solvent may include, for example, the following (the value in parentheses is the boiling point of the compound): hydrocarbon solvents such as amylbenzene (202° C.), isopropylbenzene (152° C.), 1,2-diethylbenzene (183° C.), 1,3-diethylbenzene (181° C.), 1,4-diethylbenzene (184° C.), cyclohexylbenzene (239° C.), dipentene (177° C.), 2,6-dimethylnaphthalene (262° C.), p-cymene (177° C.), camphor oil (160-185° C.), solvent naphtha (110-200° C.), cis-decalin (196° C.), trans-decalin (187° C.), decane (174° C.), tetralin (207° C.), turpentine oil (153-175° C.), kerosene (200-245° C.), dodecane (216° C.), dodecylbenzene (branched), and so forth; ketone and aldehyde solvents such as acetophenone (201.7° C.), isophorone (215.3° C.), phorone (198-199° C.), methylcyclohexanone (169.0-170.5° C.), methyl n-heptyl ketone (195.3° C.), and so forth; ester solvents such as diethyl phthalate (296.1° C.), benzyl acetate (215.5° C.), γ-butyrolactone (204° C.), dibutyl oxalate (210° C.), 2-ethylhexyl acetate (198.6° C.), ethyl benzoate (213.2° C.), benzyl formate (203° C.), and so forth; diethyl sulfate (208° C.), sulfolane (285° C.), and halohydrocarbon solvents; etherified hydrocarbon solvents; alcohol solvents; ether/acetal solvents; polyhydric alcohol solvents; carboxylic anhydride solvents; phenolic solvents; water; and silicone solvents.

60 The ratio of the mixed liquids may be established by one skilled in the art. The ratio of liquids a binary mixed liquid may be from about 1:1 to about 99:1, such as from about 1:10 to about 10:1, or about 1:5 to about 5:1, by volume. When n liquids are used, with n ranging from about 3 to 65 about 6, the amount of each liquid ranges from about 1% to about 95% such that the sum of each liquid contribution equals 100%.

In embodiments, the mixed liquid comprises at least a first and a second solvent with different boiling points. In further embodiments, the difference in boiling point between the first and the second solvent may be from about nil to about 150° C., such as from nil to about 50° C. For example, the boiling point of the first solvent may exceed the boiling point of the second solvent by about 1° C. to about 100° C., such as by about 5° C. to about 100° C., or by about 10° C. to about 50° C. The mixed liquid may comprise at least a first and a second solvent with different vapor pressures, such as combinations of high vapor pressure solvents and/or low vapor pressure solvents. The term "high vapor pressure solvent" refers to, for example, a solvent having a vapor pressure of at least about 1 kPa, such as about 2 kPa, or about 5 kPa. The term "low vapor pressure solvent" refers to, for example, a solvent having a vapor pressure of less than about 1 kPa, such as about 0.9 kPa, or about 0.5 kPa. In embodiments, the first solvent may be a low vapor pressure solvent such as, for example, terpineol, diethylene glycol, ethylene glycol, hexylene glycol, N-methyl-2-pyrrolidone, and tri(ethylene glycol) dimethyl ether. A high vapor pressure solvent allows rapid removal of the solvent by drying and/or evaporation at temperatures below the boiling point. High vapor pressure solvents may include, for example, acetone, tetrahydrofuran, toluene, xylene, ethanol, methanol, 2-butanone and water.

In embodiments Where mixed liquids comprising a first solvent, second solvent, third solvent, and so forth are used in the reaction mixture, promoting the change of the wet film and forming the dry SOF may comprise, for example, heating the wet film to a temperature above the boiling point of the reaction mixture to form the dry SOF; or heating the wet film to a temperature above the boiling point of the second solvent (below the temperature of the boiling point of the first solvent) in order to remove the second solvent while substantially leaving the first solvent and then after substantially removing the second solvent, removing the first solvent by heating the resulting composition at a temperature either above or below the boiling point of the first solvent to form the dry SOF; or heating the wet film below the boiling point of the second solvent in order to remove the second solvent (which is a high vapor pressure solvent) while substantially leaving the first solvent and, after removing the second solvent, removing the first solvent by heating the resulting composition at a temperature either above or below the boiling point of the first solvent to form the SOF.

The term "substantially removing" refers to, for example, the removal of at least 90% of the respective solvent, such as about 95% of the respective solvent. The term "substantially leaving" refers to, for example, the removal of no more than 2% of the respective solvent, such as removal of no more than 1% of the respective solvent.

These mixed liquids may be used to slow or speed up the rate of conversion of the wet layer to the SOF in order to manipulate the characteristics of the SOFs. For example, in condensation and addition/elimination linking chemistries, liquids such as water, 1°, 2°, or 3° alcohols (such as methanol, ethanol, propanol, isopropanol, butanol, 1-methoxy-2-propanol, tert-butanol) may be used.

Optionally a catalyst may be present in the reaction mixture to assist the promotion of the wet layer to the dry SOF. Selection and use of the optional catalyst depends on the functional groups on the molecular building blocks. Catalysts may be homogeneous (dissolved) or heterogeneous (undissolved or partially dissolved) and include Brönsted acids (HCl(aq), acetic acid, p-toluenesulfonic acid,

amine-protected p-toluenesulfonic acid such as pyridium p-toluenesulfonate, trifluoroacetic acid); Lewis acids (boron trifluoroetherate, aluminum trichloride); Brönsted bases (metal hydroxides such as sodium hydroxide, lithium hydroxide, potassium hydroxide; 1°, 2°, or 3° amines such as butylamine, diisopropylamine, triethylamine, diisopropylethylamine); Lewis bases (N,N-dimethyl-4-aminopyridine); metals (Cu bronze); metal salts (FeCl<sub>3</sub>, AuCl<sub>3</sub>); and metal complexes (ligated palladium complexes, ligated ruthenium catalysts). Typical catalyst loading ranges from about 0.01% to about 25%, such as from about 0.1% to about 5% of the molecular building block loading in the reaction mixture. The catalyst may or may not be present in the final SOF composition.

Optionally additives or secondary components, such as dopants, may be present in the reaction mixture and wet layer. Such additives or secondary components may also be integrated into a dry SOF. Additives or secondary components can be homogeneous or heterogeneous in the reaction mixture and wet layer or in a dry SOF. In contrast to capping units, the terms "additive" or "secondary component," refer, for example, to atoms or molecules that are not covalently bound in the SOF, but are randomly distributed in the composition. Suitable secondary components and additives are described in U.S. patent application Ser. No. 12/716,324, entitled "Composite Structured Organic Films," the disclosure of which is totally incorporated herein by reference in its entirety.

In embodiments, the secondary components may have similar or disparate properties to accentuate or hybridize (synergistic effects or ameliorative effects as well as the ability to attenuate inherent or inclined properties of the capped SOF) the intended property of the capped SOF to enable it to meet performance targets. For example, doping the capped SOFs with antioxidant compounds will extend the life of the capped SOF by preventing chemical degradation pathways. Additionally, additives maybe added to improve the morphological properties of the capped SOF by tuning the reaction occurring during the promotion of the change of the reaction mixture to form the capped SOF.

#### Process Action B: Depositing the Reaction Mixture as a Wet Film

The reaction mixture may be applied as a wet film to a variety of substrates using a number of liquid deposition techniques. The thickness of the SOF is dependant on the thickness of the wet film and the molecular building block loading in the reaction mixture. The thickness of the wet film is dependent on the viscosity of the reaction mixture and the method used to deposit the reaction mixture as a wet film.

Substrates include, for example, polymers, papers, metals and metal alloys, doped and undoped forms of elements from Groups III-VI of the periodic table, metal oxides, metal chalcogenides, and previously prepared SOFs or capped SOFs. Examples of polymer film substrates include polyesters, polyolefins, polycarbonates, polystyrenes, polyvinylchloride, block and random copolymers thereof, and the like. Examples of metallic surfaces include metallized polymers, metal foils, metal plates; mixed material substrates such as metals patterned or deposited on polymer, semiconductor, metal oxide, or glass substrates. Examples of substrates comprised of doped and undoped elements from Groups of the periodic table include, aluminum, silicon, silicon n-doped with phosphorous, silicon p-doped with boron, tin, gallium arsenide, lead, gallium indium phosphide, and indium. Examples of metal oxides include silicon dioxide, titanium dioxide, indium tin oxide, tin dioxide, selenium dioxide, and alumina. Examples of metal chalco-

genides include cadmium sulfide, cadmium telluride, and zinc selenide. Additionally, it is appreciated that chemically treated or mechanically modified forms of the above substrates remain within the scope of surfaces which may be coated with the reaction mixture.

In embodiments, the substrate may be composed of, for example, silicon, glass plate, plastic film or sheet. For structurally flexible devices, a plastic substrate such as polyester, polycarbonate, polyimide sheets and the like may be used. The thickness of the substrate may be from around 10 micrometers to over 10 millimeters with an exemplary thickness being from about 50 to about 100 micrometers, especially for a flexible plastic substrate, and from about 1 to about 10 millimeters for a rigid substrate such as glass or silicon.

The reaction mixture may be applied to the substrate using a number of liquid deposition techniques including, for example, spin coating, blade coating, web coating, dip coating, cup coating, rod coating, screen printing, ink jet printing, spray coating, stamping and the like. The method used to deposit the wet layer depends on the nature, size, and shape of the substrate and the desired wet layer thickness. The thickness of the wet layer can range from about 10 nm to about 5 mm, such as from about 100 nm to about 1 mm, or from about 1  $\mu$ m to about 500  $\mu$ m.

In embodiments, the capping unit and/or secondary component may be introduced following completion of the above described process action B. The incorporation of the capping unit and/or secondary component in this way may be accomplished by any means that serves to distribute the capping unit and/or secondary component homogeneously, heterogeneously, or as a specific pattern over the wet film. Following introduction of the capping unit and/or secondary component subsequent process actions may be carried out resuming with process action C.

For example, following completion of process action B (i.e., after the reaction mixture may be applied to the substrate), capping unit(s) and/or secondary components (dopants, additives, etc.) may be added to the wet layer by any suitable method, such as by distributing (e.g., dusting, spraying, pouring, sprinkling, etc, depending on whether the capping unit and/or secondary component is a particle, powder or liquid) the capping unit(s) and/or secondary component on the top the wet layer. The capping units and/or secondary components may be applied to the formed wet layer in a homogeneous or heterogeneous manner, including various patterns, wherein the concentration or density of the capping unit(s) and/or secondary component is reduced, in specific areas, such as to form a pattern of alternating bands of high and low concentrations of the capping unit(s) and/or secondary component of a given width on the wet layer. In embodiments, the application of the capping unit(s) and/or secondary component to the top of the wet layer may result in a portion of the capping unit(s) and/or secondary component diffusing or sinking into the wet layer and thereby forming a heterogeneous distribution of capping unit(s) and/or secondary component within the thickness of the SOF, such that a linear or nonlinear concentration gradient may be obtained in the resulting SOF obtained after promotion of the change of the wet layer to a dry SOF. In embodiments, a capping unit(s) and/or secondary component may be added to the top surface of a deposited wet layer, which upon promotion of a change in the wet film, results in an SOF having an heterogeneous distribution of the capping unit(s) and/or secondary component in the dry SOF. Depending on the density of the wet film and the density of the capping unit(s) and/or secondary component,

a majority of the capping unit(s) and/or secondary component may end up in the upper half (which is opposite the substrate) of the dry SOF or a majority of the capping unit(s) and/or secondary component may end up in the lower half (which is adjacent to the substrate) of the dry SOF.

Process Action C: Promoting the Change of Wet Film to the Dry SOF

The term "promoting" refers, for example, to any suitable technique to facilitate a reaction of the molecular building blocks, such as a chemical reaction of the functional groups of the building blocks. In the case where a liquid needs to be removed to form the dry film, "promoting" also refers to removal of the liquid. Reaction of the capping units, and molecular building blocks, and removal of the liquid can occur sequentially or concurrently. In embodiments, the capping unit may be added while the promotion of the change of the wet film to the dry SOF is occurring. In certain embodiments, the liquid is also one of the molecular building blocks and is incorporated into the SOF. The term "dry SOF" refers, for example, to substantially dry SOFs (such as capped SOFs), for example; to a liquid content less than about 5% by weight of the SOF, or to a liquid content less than 2% by weight of the SOF.

In embodiments, the dry SOF or a given region of the dry SOF (such as the surface to a depth equal to of about 10% of the thickness of the SOF or a depth equal to of about 5% of the thickness of the SOF, the upper quarter of the SOF, or the regions discussed above) the capping units are present in an amount equal to or greater than about 0.5%, by mole, with respect to the total moles of capping units and segments present, such as from about 1% to about 40%, or from about 2% to 25% by mole, with respect to the total moles of capping units and segments present. For example when the capping units are present in an amount of about 0.5% by mole respect to the total moles of capping units and segments present, there would be about 0.05 mols of capping units and about 9.95 mols of segments present in the sample.

Promoting the wet layer to form a dry SOF may be accomplished by any suitable technique. Promoting the wet layer to form a dry SOF typically involves thermal treatment including, for example, oven drying, infrared radiation (IR), and the like with temperatures ranging from 40 to 350° C. and from 60 to 200° C. and from 85 to 160° C. The total heating time can range from about four seconds to about 24 hours, such as from one minute to 120 minutes, or from three minutes to 60 minutes.

IR promotion of the wet layer to the COF film may be achieved using an IR heater module mounted over a belt transport system. Various types of IR emitters may be used, such as carbon IR emitters or short wave IR emitters (available from Heraeus). Additional exemplary information regarding carbon IR emitters or short wave IR emitters is summarized in the following Table.

| IR lamp    | Peak Wavelength | Number of lamps | Module Power (kW) |
|------------|-----------------|-----------------|-------------------|
| Carbon     | 2.0 micron      | 2-twin tube     | 4.6               |
| Short wave | 1.2-1.4 micron  | 2-twin tube     | 4.5               |

Process Action D: Optionally Removing the Capped SOF from the Coating Substrate to Obtain a Free-Standing Capped SOF

In embodiments, a free-standing SOF is desired. Free-standing capped SOFs may be obtained when an appropriate low adhesion substrate is used to support the deposition of the wet layer. Appropriate substrates that have low adhesion

to the SOF may include, for example, metal foils, metalized polymer substrates, release papers and SOFs, such as SOFs prepared with a surface that has been altered to have a low adhesion or a decreased propensity for adhesion or attachment. Removal of the SOF from the supporting substrate may be achieved in a number of ways by someone skilled in the art. For example, removal of the SOF from the substrate may occur by starting from a corner or edge of the film and optionally assisted by passing the substrate and SOF over a curved surface.

**Process Action E: Optionally Processing the Free-Standing SOF into a Roll**

Optionally, a free-standing SOF or a SOF supported by a flexible substrate may be processed into a roll. The SOF may be processed into a roll for storage, handling, and a variety of other purposes. The starting curvature of the roll is selected such that the SOF is not distorted or cracked during the rolling process.

**Process Action F: Optionally Cutting and Seaming the SOF into a Shape, Such as a Belt**

The method for cutting and seaming the SOF is similar to that described in U.S. Pat. No. 5,455,136 issued on Oct. 3<sup>rd</sup>, 1995 (for polymer films), the disclosure of which is herein totally incorporated by reference. An SOF belt may be fabricated from a single SOF, a multi layer SOF or an SOF sheet cut from a web. Such sheets may be rectangular in shape or any particular shape as desired. All sides of the SOF(s) may be of the same length, or one pair of parallel sides may be longer than the other pair of parallel sides. The SOF(s) may be fabricated into shapes, such as a belt by overlap joining the opposite marginal end regions of the SOF sheet. A seam is typically produced in the overlapping marginal end regions at the point of joining. Joining may be affected by any suitable means. Typical joining techniques include, for example, welding (including ultrasonic), gluing, taping, pressure heat fusing and the like. Methods, such as Ultrasonic welding, are desirable general methods of joining flexible sheets because of their speed, cleanliness (no solvents) and production of a thin and narrow seam.

**Process Action G: Optionally Using a SOF as a Substrate for Subsequent SOF Formation Processes**

A SOF may be used as a substrate in the SOF forming process to afford a multi-layered structured organic film. The layers of a multi-layered SOF may be chemically bound in or in physical contact. Chemically bound, multi-layered SOFs are formed when functional groups present on the substrate SOF surface can react with the molecular building blocks present in the deposited wet layer used to form the second structured organic film layer. Multi-layered SOFs in physical contact may not chemically bound to one another.

A SOF substrate may optionally be chemically treated prior to the deposition of the wet layer to enable or promote chemical attachment of a second SOF layer to form a multi-layered structured organic film.

Alternatively, a SOF substrate may optionally be chemically treated prior to the deposition of the wet layer to disable chemical attachment of a second SOF layer (surface pacification) to form a physical contact multi-layered SOF.

Other methods, such as lamination of two or more SOFs, may also be used to prepare physically contacted multi-layered SOFs.

**Applications of SOFs in Imaging Members, Such as Photoreceptor Layers**

Representative structures of an electrophotographic imaging member (e.g., a photoreceptor) are shown in FIGS. 2-4. These imaging members are provided with an anti-curl layer 1, a supporting substrate 2, an electrically conductive ground

plane 3, a charge blocking layer 4, an adhesive layer 5, a charge generating layer 6, a charge transport layer 7, an overcoating layer 8, and a ground strip 9. In FIG. 4, imaging layer 10 (containing both charge generating material and charge transport material) takes the place of separate charge generating layer 6 and charge transport layer 7.

As seen in the figures, in fabricating a photoreceptor, a charge generating material (CGM) and a charge transport material (CTM) may be deposited onto the substrate surface 10 either in a laminate type configuration where the CGM and CTM are in different layers (e.g., FIGS. 2 and 3) or in a single layer configuration where the CGM and CTM are in the same layer (e.g., FIG. 4). In embodiments, the photoreceptors may be prepared by applying over the electrically conductive layer the charge generation layer 6 and, optionally, a charge transport layer 7. In embodiments, the charge generation layer and, when present, the charge transport layer, may be applied, in either order.

**Anti Curt Layer**

20 For some applications, an optional anti-curl layer 1, which comprises film-forming organic or inorganic polymers that are electrically insulating or slightly semi-conductive, may be provided. The anti-curl layer provides flatness and/or abrasion resistance.

25 Anti-curl layer 1 may be formed at the back side of the substrate 2, opposite the imaging layers. The anti-curl layer may include, in addition to the film-forming resin, an adhesion promoter polyester additive. Examples of film-forming resins useful as the anti-curl layer include, but are not limited to, polyacrylate, polystyrene, poly(4,4'-isopropylidene diphenylcarbonate), poly(4,4'-cyclohexylidene diphenylcarbonate), mixtures thereof and the like.

30 Additives may be present in the anti-curl layer in the range of about 0.5 to about 40 weight percent of the anti-curl layer. Additives include organic and inorganic particles that may further improve the wear resistance and/or provide charge relaxation property. Organic particles include Teflon powder, carbon black, and graphite particles. Inorganic particles include insulating and semiconducting metal oxide particles such as silica, zinc oxide, tin oxide and the like. Another semiconducting additive is the oxidized oligomer salts as described in U.S. Pat. No. 5,853,906. The oligomer salts are oxidized N,N, N',N'-tetra-p-tolyl-4,4'-biphenyl-diamine salt.

35 40 Typical adhesion promoters useful as additives include, but are not limited to, duPont 49,000 (duPont), Vitel PE-100, Vitel PE-200, Vitel PE-307 (Goodyear), mixtures thereof and the like. Usually from about 1 to about 15 weight percent adhesion promoter is selected for film-forming, resin addition, based on the weight of the film-forming resin.

45 The thickness of the anti-curl layer is typically from about 3 micrometers to about 35 micrometers, such as from about 10 micrometers to about 20 micrometers, or about 14 micrometers.

50 55 The anti-curl coating may be applied as a solution prepared by dissolving the film-forming, resin and the adhesion promoter in a solvent such as methylene chloride. The solution may be applied to the rear surface of the supporting substrate (the side opposite the imaging layers) of the photoreceptor device, for example, by web coating or by other methods known in the art. Coating of the overcoat layer and the anti-curl layer may be accomplished simultaneously by web coating onto a multilayer photoreceptor comprising a charge transport layer, charge generation layer, adhesive layer blocking layer, ground plane and substrate. The wet film coating is then dried to produce the anti-curl layer 1.

## The Supporting Substrate

As indicated above, the photoreceptors are prepared by first providing a substrate 2, i.e., a support. The substrate may be opaque or substantially transparent and may comprise any additional suitable material(s) having given required mechanical properties, such as those described in U.S. Pat. Nos. 4,457,994; 4,871,634; 5,702,854; 5,976,744; and 7,384,717 the disclosures of which are incorporated herein by reference in their entireties.

The substrate may comprise a layer of electrically non-conductive material or a layer of electrically conductive material, such as an inorganic or organic composition. If a non-conductive material is employed, it may be necessary to provide an electrically conductive ground plane over such non-conductive material. If a conductive material is used as the substrate, a separate ground plane layer may not be necessary.

The substrate may be flexible or rigid and may have any of a number of different configurations, such as, for example, a sheet, a scroll, an endless flexible belt, a web, a cylinder, and the like. The photoreceptor may be coated on a rigid, opaque, conducting substrate, such as an aluminum drum.

Various resins may be used as electrically non-conducting materials, including, for example, polyesters, polycarbonates, polyamides, polyurethanes, and the like. Such a substrate may comprise a commercially available biaxially oriented polyester known as MYLARTM, available from E.I. duPont de Nemours & Co., MELINEXTM, available from ICI Americas Inc., or HOSTAPHANTM, available from American Hoechst Corporation. Other materials of which the substrate may be comprised include polymeric materials, such as polyvinyl fluoride, available as TEDLARTM from E.I. duPont de Nemours & Co., polyethylene and polypropylene, available as MARLEXTM from Phillips Petroleum Company, polyphenylene sulfide, RYTONTM available from Phillips Petroleum Company, and polyimides, available as KAPONTM from E.I. duPont de Nemours & Co. The photoreceptor may also be coated on an insulating plastic drum, provided a conducting ground plane has previously been coated on its surface, as described above. Such substrates may either be seamed or seamless.

When a conductive substrate is employed, any suitable conductive material may be used. For example, the conductive material can include, but is not limited to, metal flakes, powders or fibers, such as aluminum, titanium, nickel, chromium, brass, gold, stainless steel, carbon black, graphite, or the like, in a binder resin including metal oxides, sulfides, silicides, quaternary ammonium salt compositions, conductive polymers such as polyacetylene or its pyrolysis and molecular doped products, charge transfer complexes, and polyphenyl silane and molecular doped products from polyphenyl silane. A conducting plastic drum may be used, as well as the conducting metal drum made from a material such as aluminum.

The thickness of the substrate depends on numerous factors, including the required mechanical performance and economic considerations. The thickness of the substrate is typically within a range of from about 65 micrometers to about 150 micrometers, such as from about 75 micrometers to about 125 micrometers for optimum flexibility and minimum induced surface bending stress when cycled around small diameter rollers, e.g., 19 mm diameter rollers. The substrate for a flexible belt may be of substantial thickness, for example, over 200 micrometers, or of minimum thickness, for example, less than 50 micrometers, provided there are no adverse effects on the final photoconductive device.

Where a drum is used, the thickness should be sufficient to provide the necessary rigidity. This is usually about 1-6 mm.

The surface of the substrate to which a layer is to be applied may be cleaned to promote greater adhesion of such a layer. Cleaning may be effected, for example, by exposing the surface of the substrate layer to plasma discharge, ion bombardment, and the like. Other methods, such as solvent cleaning, may also be used.

10 Regardless of any technique employed to form a metal layer, a thin layer of metal oxide generally forms on the outer surface of most metals upon exposure to air. Thus, when other layers overlying the metal layer are characterized as "contiguous" layers, it is intended that these overlying contiguous layers may, in fact, contact a thin metal oxide layer that has formed on the outer surface of the oxidizable metal layer.

## The Electrically Conductive Ground Plane

As stated above, in embodiments, the photoreceptors 20 prepared comprise a substrate that is either electrically conductive or electrically non-conductive. When a non-conductive substrate is employed, an electrically conductive ground plane 3 must be employed, and the ground plane acts as the conductive layer. When a conductive substrate is employed, the substrate may act as the conductive layer, although a conductive ground plane may also be provided.

If an electrically conductive ground plane is used, it is positioned over the substrate. Suitable materials for the electrically conductive ground plane include, for example, 30 aluminum, zirconium, niobium, tantalum, vanadium, hafnium, titanium, nickel, stainless steel, chromium, tungsten, molybdenum, copper, and the like, and mixtures and alloys thereof. In embodiments, aluminum, titanium, and zirconium may be used.

35 The ground plane may be applied by known coating techniques, such as solution coating, vapor deposition, and sputtering. A method of applying an electrically conductive ground plane is by vacuum deposition. Other suitable methods may also be used.

40 In embodiments, the thickness of the ground plane may vary over a substantially wide range, depending on the optical transparency and flexibility desired, for the electrophotoconductive member. For example, for a flexible photoreponsive imaging device, the thickness of the conductive layer may be between about 20 angstroms and about 750 angstroms; such as, from about 50 angstroms to about 200 angstroms for an optimum combination of electrical conductivity, flexibility, and light transmission. However, the ground plane can, if desired, be opaque.

## The Charge Blocking Layer

45 After deposition of any electrically conductive ground plane layer, a charge blocking layer 4 may be applied thereto. Electron blocking layers for positively charged photoreceptors permit holes from the imaging surface of the 55 photoreceptor to migrate toward the conductive layer. For negatively charged photoreceptors, any suitable hole blocking layer capable of forming a barrier to prevent hole injection from the conductive layer to the opposite photoconductive layer may be utilized.

60 If a blocking layer is employed, it may be positioned over the electrically conductive layer. The term "over," as used herein in connection with many different types of layers, should be understood as not being limited to instances wherein the layers are contiguous. Rather, the term "over" 65 refers, for example, to the relative placement of the layers and encompasses the inclusion of unspecified intermediate layers.

The blocking layer **4** may include polymers such as polyvinyl butyral, epoxy resins, polyesters, polysiloxanes, polyamides, polyurethanes, and the like; nitrogen-containing siloxanes or nitrogen-containing titanium compounds, such as trimethoxysilyl propyl ethylene diamine, N-beta (aminoethyl) gamma-aminopropyl trimethoxy silane, isopropyl 4-aminobenzene sulfonyl titanate, di(dodecylbenzene sulfonyl) titanate, isopropyl di(4-aminobenzoyl) isostearoyl titanate, isopropyl tri(N-ethyl amino) titanate, isopropyl trianthranil titanate, isopropyl tri(N,N-dimethyl-ethyl amino) titanate, titanium-4-amino benzene sulfonate oxyacetate, titanium 4-aminobenzoate isostearate oxyacetate, gamma-aminobutyl methyl dimethoxy silane, gamma-aminopropyl methyl dimethoxy silane, and gamma-aminopropyl trimethoxy silane, disclosed in U.S. Pat. Nos. 4,338,387; 4,286,033; and 4,291,110 the disclosures of which are incorporated herein by reference in their entireties.

The blocking layer may be continuous and may have a thickness ranging, for example, from about 0.01 to about 10 micrometers, such as from about 0.05 to about 5 micrometers.

The blocking layer **4** may be applied by any suitable technique, such as spraying, dip coating, draw bar coating, gravure coating, silk screening, air knife coating, reverse roll coating, vacuum deposition, chemical treatment, and the like. For convenience in obtaining thin layers, the blocking layer may be applied in the form of a dilute solution, with the solvent being removed after deposition of the coating by conventional techniques, such as by vacuum, heating, and the like. Generally, a weight ratio of blocking layer material and solvent of between about 0.5:100 to about 30:100, such as about 5:100 to about 20:100, is satisfactory for spray and dip coating.

The present disclosure further provides a method for forming the electrophotographic photoreceptor, in which the charge blocking layer is formed by using a coating solution composed of the grain shaped particles, the needle shaped particles, the binder resin and an organic solvent.

The organic solvent may be a mixture of an azeotropic mixture of C<sub>1-3</sub> lower alcohol and another organic solvent selected from the group consisting of dichloromethane, chloroform, 1,2-dichloroethane, 1,2-dichloropropane, toluene and tetrahydrofuran. The azeotropic mixture mentioned above is a mixture solution in which a composition of the liquid phase and a composition of the vapor phase are coincided with each other at a certain pressure to give a mixture having a constant boiling point. For example, a mixture consisting of 35 parts by weight of methanol and 65 parts by weight of 1,2-dichloroethane is an azeotropic solution. The presence of an azeotropic composition leads to uniform evaporation, thereby forming a uniform charge blocking layer without coating defects and improving storage stability of the charge blocking coating solution.

The binder resin contained in the blocking layer may be formed of the same materials as that of the blocking layer formed as a single resin layer. Among them, polyamide resin may be used because it satisfies various conditions required of the binder resin such as (i) polyamide resin is neither dissolved nor swollen in a solution used for forming the imaging layer on the blocking layer, and (ii) polyamide resin has an excellent adhesiveness with a conductive support as well as flexibility. In the polyamide resin, alcohol soluble nylon resin may be used, for example, copolymer nylon polymerized with 6-nylon, 6,6-nylon, 610-nylon, 11-nylon, 12-nylon and the like; and nylon which is chemically denatured such as N-alkoxy methyl denatured nylon and

N-alkoxy ethyl denatured nylon. Another type of binder resin that may be used is a phenolic resin or polyvinyl butyral resin.

The charge blocking layer is formed by dispersing the hinder resin, the grain shaped particles, and the needle shaped particles in the solvent to form a coating solution for the blocking layer; coating the conductive support with the coating solution and drying it. The solvent is selected for improving dispersion in the solvent and for preventing the coating solution from gelation with the elapse of time. Further, the azeotropic solvent may be used for preventing the composition of the coating solution from being changed as time passes, whereby storage stability of the coating solution may be improved and the coating solution may be reproduced.

The phrase "n-type" refers, for example, to materials which predominately transport electrons. Typical n-type materials include dibromoanthanthrone, benzimidazole perylene, zinc oxide, titanium oxide, azo compounds such as chlorodiane Blue and bisazo pigments, substituted 2,4-dibroroniazines, polynuclear aromatic quinones, zinc sulfide, and the like.

The phrase "p-type" refers, for example, to materials which transport holes. Typical p-type organic pigments include, for example, metal-free phthalocyanine, titanyl phthalocyanine, gallium phthalocyanine, hydroxy phthalocyanine, chlorogallium phthalocyanine, copper phthalocyanine, and the like.

#### 30 The Adhesive Layer

An intermediate layer **5** between the blocking layer and the charge generating layer may, if desired, be provided to promote adhesion. However, in embodiments, a dip coated aluminum drum may be utilized without an adhesive layer.

35 Additionally, adhesive layers may be provided, if necessary, between any of the layers in the photoreceptors to ensure adhesion of any adjacent layers. Alternatively, or in addition, adhesive material may be incorporated into one or both of the respective layers to be adhered. Such optional adhesive layers may have thicknesses of about 0.001 micrometer to about 0.2 micrometer. Such an adhesive layer may be applied, for example, by dissolving adhesive material in an appropriate solvent, applying by hand, spraying, dip coating, draw bar coating, gravure coating, silk screening, air knife coating, vacuum deposition, chemical treatment, roll coating, wire wound rod coating, and the like, and drying to remove the solvent. Suitable adhesives include, for example, film-forming polymers, such as polyester, dupont 49,000 (available from E. I. dupont de Nemours & Co.), Vitel PE-100 (available from Goodyear Tire and Rubber Co.), polyvinyl butyral, polyvinyl pyrrolidone, polyurethane, polymethyl methacrylate, and the like. The adhesive layer may be composed of a polyester with M<sub>w</sub> of from about 50,000 to about 100,000, such as about 70,000, and a M<sub>n</sub> of about 35,000.

#### 55 The Imaging Layer(s)

The imaging layer refers to a layer or layers containing charge generating material, charge transport material, or both the charge generating material and the charge transport material.

60 Either a n-type or a p-type charge generating material may be employed in the present photoreceptor.

In the case where the charge generating material and the charge transport material are in different layers—for example a charge generation layer and a charge transport layer—the charge transport layer may comprise a SOF, which may be a capped SOF. Further, in the case where the

charge generating material and the charge transport material are in the same layer, this layer may comprise a SOF, which may be a capped SOF.

#### Charge Generation Layer

Illustrative organic photoconductive charge generating materials include azo pigments such as Sudan Red, Dian Blue, Janus Green B, and the like; quinone pigments such as Algal Yellow, Pyrene Quinone, Indanthrene Brilliant Violet RRP, and the like; quinocyanine pigments; perylene pigments such as benzimidazole perylene; indigo pigments such as indigo, thioindigo, and the like; bisbenzimidazole pigments such as Indofast Orange, and the like; phthalocyanine pigments such as copper phthalocyanine, aluminum-chlorophthalocyanine, hydroxylgallium phthalocyanine, chlorogallium phthalocyanine, titanyl phthalocyanine and the like; quinacridone pigments; or azulene compounds. Suitable inorganic photoconductive charge generating materials include for example cadmium sulfide, cadmium sulfoselenide, cadmium selenide, crystalline and amorphous selenium, lead oxide and other chalcogenides. In embodiments, alloys of selenium may be used and include for instance selenium-arsenic, selenium-tellurium-arsenic, and selenium-tellurium.

Any suitable inactive resin binder material may be employed in the charge generating layer. Typical organic resinous binders include polycarbonates, acrylate polymers, methacrylate polymers, vinyl polymers, cellulose polymers, polyesters, polysiloxanes, polyamides, polyurethanes, epoxies, polyvinylacetals, and the like.

To create a dispersion useful as a coating composition, a solvent is used with the charge generating material. The solvent may be for example cyclohexanone, methyl ethyl ketone, tetrahydrofuran, alkyl acetate, and mixtures thereof. The alkyl acetate (such as butyl acetate and amyl acetate) can have from 3 to 5 carbon atoms in the alkyl group. The amount of solvent in the composition ranges for example from about 70% to about 98% by weight, based on the weight of the composition.

The amount of the charge generating material in the composition ranges for example from about 0.5% to about 30% by weight, based on the weight of the composition including a solvent. The amount of photoconductive particles (i.e., the charge generating material) dispersed in a dried photoconductive coating varies to some extent with the specific photoconductive pigment particles selected. For example, when phthalocyanine organic pigments such as titanyl phthalocyanine and metal-free phthalocyanine are utilized, satisfactory results are achieved when the dried photoconductive coating comprises between about 30 percent by weight and about 90 percent by weight of all phthalocyanine pigments based on the total weight of the dried photoconductive coating. Because the photoconductive characteristics are affected by the relative amount of pigment per square centimeter coated, a lower pigment loading may be utilized if the dried photoconductive coating layer is thicker. Conversely, higher pigment loadings are desirable where the dried photoconductive layer is to be thinner.

Generally, satisfactory results are achieved with an average photoconductive particle size of less than about 0.6 micrometer when the photoconductive coating is applied by dip coating. The average photoconductive particle size may be less than about 0.4 micrometer. In embodiments, the photoconductive particle size is also less than the thickness of the dried photoconductive coating in which it is dispersed.

In a charge generating layer, the weight ratio of the charge generating material ("CGM") to the binder ranges from 30 (CGM):70 (binder) to 70 (CGM):30 (binder).

For multilayered photoreceptors comprising a charge generating layer (also referred herein as a photoconductive layer) and a charge transport layer, satisfactory results may be achieved with a dried photoconductive layer coating thickness of between about 0.1 micrometer and about 10 micrometers. In embodiments, the photoconductive layer thickness is between about 0.2 micrometer and about 4 micrometers. However, these thicknesses also depend upon the pigment loading. Thus, higher pigment loadings permit the use of thinner photoconductive coatings. Thicknesses outside these ranges may be selected providing the objectives of the present invention are achieved.

Any suitable technique may be utilized to disperse the photoconductive particles in the binder and solvent of the coating composition. Typical dispersion techniques include, for example, ball milling, roll milling, milling in vertical attritors, sand milling, and the like. Typical milling times using a ball roll mill is between about 4 and about 6 days.

Charge transport materials include an organic polymer, a non-polymeric material, or a SOF, which may be a capped SOF, capable of supporting the injection of photoexcited holes or transporting electrons from the photoconductive material and allowing the transport of these holes or electrons through the organic layer to selectively dissipate a surface charge.

#### Organic Polymer Charge Transport Layer

Illustrative charge transport materials include for example a positive hole transporting material selected from compounds having in the main chain or the side chain a polycyclic aromatic ring such as anthracene, pyrene, phenanthrene, coronene, and the like, or a nitrogen-containing hetero ring such as indole, carbazole, oxazole, isoxazole, thiazole, imidazole, pyrazole, oxadiazole, pyrazoline, thiadiazole, triazole, and hydrazone compounds. Typical hole transport materials include electron donor materials, such as carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole); poly(vinylpyrene); poly(vinyltetraphene); poly(vinyltetracene) and poly(vinylperylene). Suitable electron transport materials include electron acceptors such as 2,4,7-trinitro-9-fluorenone; 2,4,5,7-tetranitro-fluorenone; dinitroanthracene; dinitroacridene; tetracyanopyrene; dinitroanthraquinone; and butylcarbonylfluorenemalononitrile, see U.S. Pat. No. 4,921,769 the disclosure of which is incorporated herein by reference in its entirety. Other hole transporting materials include arylamines described in U.S. Pat. No. 4,265,990 the disclosure of which is incorporated herein by reference in its entirety, such as N,N'-diphenyl-N,N'-bis(alkylphenyl)-(1,1'-biphenyl)-4,4'-diamine wherein alkyl is selected from the group consisting of methyl, ethyl, propyl, butyl, hexyl, and the like. Other known charge transport layer molecules may be selected, reference for example U.S. Pat. Nos. 4,921,773 and 4,464,450 the disclosures of which are incorporated herein by reference in their entireties.

Any suitable inactive resin binder may be employed in the charge transport layer. Typical inactive resin binders soluble in methylene chloride include polycarbonate resin, polyvinylcarbazole, polyester, polyarylate, polystyrene, polyacrylate, polyether, polysulfone, and the like. Molecular weights can vary from about 20,000 to about 1,500,000.

In a charge transport layer, the weight ratio of the charge transport material ("CTM") to the binder ranges from 30 (CTM):70 (binder) to 70 (CTM):30 (binder).

Any suitable technique may be utilized to apply the charge transport layer and the charge generating layer to the substrate. Typical coating techniques include dip coating, roll coating, spray coating, rotary atomizers, and the like. The coating techniques may use a ride concentration of solids. The solids content is between about 2 percent by weight and 30 percent by weight based on the total weight of the dispersion. The expression "solids" refers, for example, to the charge transport particles and hinder components of the charge transport coating dispersion. These solids concentrations are useful in dip coating, roll, spray coating, and the like. Generally, a more concentrated coating dispersion may be used for roll coating. Drying of the deposited coating may be effected by any suitable conventional technique such as oven drying, infra-red radiation drying, air drying and the like. Generally, the thickness of the transport layer is between about 5 micrometers to about 100 micrometers, but thicknesses outside these ranges can also be used. In general, the ratio of the thickness of the charge transport layer to the charge generating layer is maintained, for example, from about 2:1 to 200:1 and in some instances as great as about 400:1.

#### Capped SOF Charge Transport Layer

Illustrative charge transport capped SOFs include for example a positive hole transporting material selected from compounds having a segment containing a polycyclic aromatic ring such as anthracene, pyrene, phenanthrene, coronene, and the like, or a nitrogen-containing hetero ring such as indole, carbazole, oxazole, isoxazole, thiazole, imidazole, pyrazole, oxadiazole, pyrazoline, thiadiazole, triazole, and hydrazone compounds. Typical hole transport SOF segments include electron donor materials, such as carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzo-chrysene; 2,4-benzopyrene; and 1,4-bromopyrene. Suitable electron transport SOF segments include electron acceptors such as 2,4,7-trinitro-9-fluorenone; 2,4,5,7-tetrinitro-fluorenone dinitroanthracene; dinitroacridene; tetracyanopyrene; dinitroanthraquinone; and butylcarbonylfluorenemalononitrile, see U.S. Pat. No. 4,921,769. Other hole transporting SOF segments include arylamines described in U.S. Pat. No. 4,265,990, such as N,N'-diphenyl-N,N'-bis(alkylphenyl)-(1,1'-biphenyl)-4,4'-diamine wherein alkyl is selected from the group consisting of methyl, ethyl, propyl, butyl, hexyl, and the like. Other known charge transport SOF segments may be selected, reference for example U.S. Pat. Nos. 4,921,773 and 4,464,450.

The capped SOF charge transport layer may be prepared by

- preparing a liquid-containing reaction mixture comprising a plurality of molecular building blocks with inclined charge transport properties each comprising a segment and a number of functional groups;
- depositing the reaction mixture as a wet and
- promoting a change of the wet film including the molecular building blocks to a dry film comprising the SOF comprising a plurality of the segments and a plurality of linkers arranged as a covalent organic framework, wherein at a macroscopic level the covalent organic framework is a film.

Addition of the capping unit may occur during any of the steps a, b, and c, as described above. The deposition of the

reaction mixture as a wet layer may be achieved by any suitable conventional technique and applied by any of a number of application methods. Typical application methods include, for example, hand coating, spray coating, web coating, dip coating and the like. The capped SOF forming reaction mixture may use a wide range of molecular building block loadings. In embodiments, the loading is between about 2 percent by weight and 50 percent by weight based on the total weight of the reaction mixture. The term "loading" refers, for example, to the molecular building block components of the charge transport capped SOF reaction mixture. These loadings are useful in dip coating, roll, spray coating, and the like. Generally, a more concentrated coating dispersion may be used for roll coating. Drying of the deposited coating may be affected by any suitable conventional technique such as oven drying, infra-red radiation drying, air drying and the like. Generally, the thickness of the charge transport SOF layer is between about 5 micrometers to about 100 micrometers, such as about 10 micrometers to about 70 micrometers or 10 micrometers to about 40 micrometers. In general, the ratio of the thickness of the charge transport layer to the charge generating layer may be maintained from about 2:1 to 200:1 and in some instances as great as 400:1.

#### Single Layer P/R-Organic Polymer

The materials and procedures described herein may be used to fabricate a single imaging layer type photoreceptor containing a binder, a charge generating material, and a charge transport material. For example, the solids content in the dispersion for the single imaging layer may range from about 2% to about 30% by weight, based on the weight of the dispersion.

Where the imaging layer is a single layer combining the functions of the charge generating layer and the charge transport layer, illustrative amounts of the components contained therein are as follows: charge generating material (about 5% to about 40% by weight), charge transport material (about 20% to about 60% by weight), and binder (the balance of the imaging layer).

#### Single Layer P/R-Capped SOF

The materials and procedures described herein may be used to fabricate a single imaging layer type photoreceptor containing a charge generating material and a charge transport capped SOF. For example, the solids content in the dispersion for the single imaging layer may range from about 2% to about 30% by weight, based on the weight of the dispersion.

Where the imaging layer is a single layer combining the functions of the charge generating layer and the charge transport layer, illustrative amounts of the components contained therein are as follows: charge generating material (about 2% to about 40% by weight), with an inclined added functionality of charge transport molecular building block (about 20% to about 75% by weight).

#### The Overcoating Layer

Embodiments in accordance with the present disclosure can, optional further include an overcoating layer or layers 8, which, if employed, are positioned over the charge generation layer or over the charge transport layer. This layer 60 comprises capped SOFs that are electrically insulating or slightly semi-conductive.

Such a protective overcoating layer includes a capped SOF forming reaction mixture containing a capping unit and a plurality of molecular building blocks that optionally contain charge transport segments. FIG. 5 represents a simplified schematic illustrating the formation of an outer layer of an imaging member according to the present

embodiments. As shown, the building blocks comprising hole transport moieties **15** and fluorinated building blocks **20** are used to form a fluorinated SOF having hole transport molecule capping units. As depicted, R is a hole transport moiety and R—OH together is a hole transport molecule capping unit. On the right hand side, the film structure at the molecular level is shown. As shown, there are interruptions in the network and hole transport molecule capping units. This fluorinated SOF comprising hole transport molecule capping units may also be used as an imaging layer, such as the charge transport layer.

Additives may be present in the overcoating layer in the range of about 0.5 to about 40 weight percent of the overcoating layer. In embodiments, additives include organic and inorganic particles which can further improve the wear resistance and/or provide charge relaxation property. In embodiments, organic particles include Teflon powder, carbon black, and graphite particles. In embodiments, inorganic particles include insulating and semiconducting metal oxide particles such as silica, zinc oxide, tin oxide and the like. Another semiconducting additive is the oxidized oligomer salts as described in U.S. Pat. No. 5,853,906 the disclosure of which is incorporated herein by reference in its entirety. In embodiments, oligomer salts are oxidized N,N, N',N'-tetra-p-tolyl-4,4'-biphenyldiamine salt.

The capped SOF overcoating layer may be prepared by:

- preparing a liquid-containing reaction mixture comprising a plurality of molecular building blocks with an inclined charge transport properties each comprising a segment and a number of functional groups;
- depositing the reaction mixture as a wet film; and
- promoting a change of the wet film including the molecular building blocks to a dry film comprising the SOF comprising a plurality of the segments and a plurality of linkers arranged as a covalent organic framework, wherein at a macroscopic level the covalent organic framework is a film.

Addition of the capping unit may occur during any of the steps a, b, and c, as described above. The deposition of the reaction mixture as a wet layer may be achieved by any suitable conventional technique and applied by any of a number of application methods. Typical application methods include, for example, hand coating, spray coating, web coating, dip coating and the like. Promoting the change of the wet film to the dry SOF may be affected by any suitable conventional techniques, such as oven drying, infrared radiation drying, air drying, and the like.

Overcoating layers from about 2 micrometers to about 15 micrometers, such as from about 3 micrometers to about 8 micrometers are effective in preventing charge transport molecule leaching, crystallization, and charge transport layer cracking in addition to providing scratch and wear resistance.

#### The Ground Strip

The ground strip **9** may comprise a film-forming binder and electrically conductive particles. Cellulose may be used to disperse the conductive particles. Any suitable electrically conductive particles may be used in the electrically conductive ground strip layer **8**. The ground strip **8** may, for example, comprise materials that include those enumerated in U.S. Pat. No. 4,664,995 the disclosure of which is incorporated herein by reference in its entirety. Typical electrically conductive particles include, for example, carbon black, graphite, copper, silver, gold, nickel, tantalum, chromium, zirconium, vanadium, niobium, indium tin oxide, and the like.

The electrically conductive particles may have any suitable shape. Typical shapes include irregular, granular, spherical, elliptical, cubic, flake, filament, and the like. In embodiments, the electrically conductive particles should have a particle size less than the thickness of the electrically conductive ground strip layer to avoid an electrically conductive ground strip layer having an excessively irregular outer surface. An average particle size of less than about 10 micrometers generally avoids excessive protrusion of the electrically conductive particles at the outer surface of the dried ground strip layer and ensures relatively uniform dispersion of the particles through the matrix of the dried ground strip layer. Concentration of the conductive particles to be used in the ground strip depends on factors such as the conductivity of the specific conductive materials utilized.

In embodiments, the ground strip layer may have a thickness of from about 7 micrometers to about 42 micrometers, such as from about 14 micrometers to about 27 micrometers.

In embodiments, an imaging member may comprise a capped SOF as the surface layer (OCL or CTL). This imaging member may be a capped SOF that comprises N,N,N',N'-tetra-(methylenephylene)biphenyl-4,4'-diamine and segments N,N,N',N'-tetraphenyl-terphenyl-4,4'-diamine segments. Such an capped SOF may be prepared from N,N,N',N'-tetrakis-[(4-hydroxymethyl)phenyl]-biphenyl-4,4'-diamine and N,N'-diphenyl-N,N'-bis-(3-hydroxyphenyl)-terphenyl-4,4'-diamine molecular building blocks. The SOF imaging member may also comprise N,N,N',N'-tetra-(methylenephylene)biphenyl-4,4'-diamine and segments N,N,N',N'-tetraphenyl-biphenyl-4,4'-diamine segments. In embodiments, the SOF of the imaging member may be prepared from N,N,N',N'-tetrakis-[(4-hydroxymethyl)phenyl]-biphenyl-4,4'-diamine and N,N'-diphenyl-N,N'-bis-(3-hydroxyphenyl)-biphenyl-4,4'-diamine molecular building blocks.

In embodiments, imaging member may comprise a SOF, which may be a capped SOF layer, where the thickness of the SOF layer is between 1 and 15 microns. The SOF, which may be a capped SOF, in such an imaging member may be a single layer or two or more layers.

In embodiments, a SOF and/or capped SOF may be incorporated into various components of an image forming apparatus. For example, a SOF and/or capped SOF may be incorporated into a electrophotographic photoreceptor, a contact charging device, an exposure device, a developing device, a transfer device and/or a cleaning unit. In embodiments, such an image forming apparatus may be equipped with an image fixing device, and, a medium to which an image is to be transferred is conveyed to the image fixing device through the transfer device.

The contact charging device may have a roller-shaped contact charging member. The contact charging member may be arranged so that it comes into contact with a surface of the photoreceptor, and a voltage is applied, thereby being able to give a specified potential to the surface of the photoreceptor. In embodiments, a contact charging member may be formed from a SOF and/or capped SOF and/or a metal such as aluminum, iron or copper, a conductive polymer material such as a polyacetylene, a polypyrrole or a polythiophene, or a dispersion of fine particles of carbon black, copper iodide, silver iodide, zinc sulfide, silicon carbide, a metal oxide or the like in an elastomer material such as polyurethane rubber, silicone rubber, epichlorohydrin rubber, ethylene-propylene rubber, acrylic rubber, fluororubber, styrene-butadiene rubber or butadiene rubber.

Further, a covering layer, optionally comprising an SOF, may also be provided on a surface of the contact charging member of embodiments. In order to further adjust resistivity, the SOF may be a composite SOF or a capped SOF or a combination thereof, and in order to prevent deterioration, the SOF may be tailored to comprise an antioxidant either bonded or added thereto.

The resistance of the contact-charging member of embodiments may in any desired range, such as from about  $10^0$  to about  $10^{14}$   $\Omega$ cm, or from about  $10^2$  to about  $10^{12}$   $\Omega$ cm. When a voltage is applied to this contact-charging member, either a DC voltage or an AC voltage may be used as the applied voltage. Further, a superimposed voltage of a DC voltage and an AC voltage may also be used.

In an exemplary apparatus, the contact-charging member, optionally comprising an SOF, such as a capped SOF, of the contact-charging device may be in the shape of a roller. However, such a contact-charging member may also be in the shape of a blade, a belt, a brush or the like.

In embodiments an optical device that can perform desired imagewise exposure to a surface of the electrophotographic photoreceptor with a light source such as a semiconductor laser, an LED (light emitting diode) or a liquid crystal shutter, may be used as the exposure device.

In embodiments, a known developing device using a normal or reversal developing agent of a one-component system, a two-component system or the like may be used in embodiments as the developing device. There is no particular limitation on image forming material (such as a toner, ink or the like, liquid or solid) that may be used in embodiments of the disclosure.

Contact type transfer charging devices using a belt, a roller, a film, a rubber blade or the like, or a scorotron transfer charger or a scorotron transfer charger utilizing corona discharge may be employed as the transfer device, in various embodiments. In embodiments, the charging unit may be a biased charge roll, such as the biased charge rolls described in U.S. Pat. No. 7,177,572 entitled "A Biased Charge Roller with Embedded Electrodes with Post-Nip Breakdown to Enable Improved Charge Uniformity," the total disclosure of which is hereby incorporated by reference in its entirety.

Further, in embodiments, the cleaning device may be a device for removing a remaining image forming material, such as a toner or ink (liquid or solid), adhered to the surface of the electrophotographic photoreceptor after a transfer step, and the electrophotographic photoreceptor repeatedly subjected to the above-mentioned image formation process may be cleaned thereby. In embodiments, the cleaning device may be a cleaning blade, a cleaning brush, a cleaning roll or the like. Materials for the cleaning blade include SOFs or urethane rubber, neoprene rubber and silicone rubber.

In an exemplary image forming device, the respective steps of charging, exposure, development, transfer and cleaning are conducted in turn in the rotation step of the electrophotographic photoreceptor, thereby repeatedly performing image formation. The electrophotographic photoreceptor may be provided with specified layers comprising SOFs and photosensitive layers that comprise the desired SOF, and thus photoreceptors having excellent discharge gas resistance, mechanical strength, scratch resistance, particle dispersibility, etc., may be provided. Accordingly, even in embodiments in which the photoreceptor is used together with the contact charging device or the cleaning blade, or further with spherical toner obtained by chemical polymerization, good image quality may be obtained without the

occurrence of image defects such as fogging. That is, embodiments of the invention provide image-forming apparatuses that can stably provide good image quality for a long period of time is realized.

A number of examples of the process used to make SOFs and, capped SOFs are set forth herein and are illustrative of the different compositions, conditions, techniques that may be utilized. Identified within each example are the nominal actions associated with this activity. The sequence and number of actions along with operational parameters, such as temperature, time, coating method, and the like, are not limited by the following examples. All proportions are by weight unless otherwise indicated. The term "rt" refers, for example, to temperatures ranging from about 20° C., to about 25° C. Mechanical measurements were measured on a TA Instruments DMA Q800 dynamic mechanical analyzer using methods standard in the art. Differential scanning calorimetry was measured on a TA Instruments DSC 2910 differential scanning calorimeter using methods standard in the art. Thermal gravimetric analysis was measured on a TA Instruments TGA 2950 thermal gravimetric analyzer using methods standard in the art. FT-IR spectra was measured on a Nicolet Magna 550 spectrometer using methods standard in the art. Thickness measurements <1 micron were measured on a Dektak 6m Surface Profiler. Surface energies were measured on a Fibro DAT 1100 (Sweden) contact angle instrument using methods standard in the art. Unless otherwise noted, the SOFs produced in the following examples were either pinhole-free SOFs or substantially pinhole-free SOFs.

The SOFs coated onto Mylar were delaminated by immersion in a room temperature water bath. After soaking for 10 minutes the SOF generally detached from Mylar substrate. This process is most efficient with a SOF coated onto substrates known to have high surface energy (polar), such as glass, mica, salt, and the like.

Given the examples below it will be apparent, that the compositions prepared by the methods of the present disclosure may be practiced with many types of components and may have many different uses in accordance with the disclosure above and as pointed out hereinafter.

The SOF capping units may also be added to an SOF wherein the microscopic arrangement of segments is patterned. The term "patterning" refers, for example, to the sequence in which segments are linked together.

A patterned film may be detected using spectroscopic techniques that are capable of assessing the successful formation of linking groups in a SOF. Such spectroscopies include, for example, Fourier-transfer infrared spectroscopy, Raman spectroscopy, and solid-state nuclear magnetic resonance spectroscopy. Upon acquiring a data by a spectroscopic technique from a sample, the absence of signals from functional groups on building blocks and the emergence of signals from linking groups indicate the reaction between building blocks and the concomitant patterning and formation of an SOF.

Different degrees of patterning are also embodied. Full patterning of a SOF will be detected by the complete absence of spectroscopic signals from building block functional groups. Also embodied are SOFs having lowered degrees of patterning wherein domains of patterning exist within the SOF. SOFs with domains of patterning, when measured spectroscopically, will produce signals from building block functional groups which remain unmodified at the periphery of a patterned domain.

It is appreciated that a very low degree of patterning is associated with inefficient reaction between building blocks

and the inability to form a film. Therefore, successful implementation of the process of the present disclosure requires appreciable patterning between building blocks within the SOF. The degree of necessary patterning to form a SOF is variable and can depend on the chosen capping units, building blocks and desired linking groups. The minimum degree of patterning required is that required to form a film using the process described herein, and may be quantified as formation of about 20% or more of the intended linking groups, such as about 40% or more of the intended linking groups or about 50% or more of the intended linking groups. Formation of linking groups and capping units may be detected spectroscopically as described earlier in the embodiments.

#### Mechanical/Chemical Properties

In embodiments some capped SOFs are found to have different toughness (FIG. 8). By introduction of capping units, and varying capping group concentration in a SOF, the toughness of the SOF can be enhanced or the toughness of the SOF can be attenuated.

In embodiments, toughness may be assessed by measuring the stress-strain curve for SOFs. This test is conducted by mounting a dog-bone shaped piece of SOF of known dimensions between two clamps; one stationary, and one moving. The moving clamp applies a force at a known rate (N/min) causing a stress (Force/area) on the film. This stress causes the film to elongate and a graph comparing stress vs. strain is created. The Young's Modulus (slope of the linear section) as well as rupture point (stress and strain at breakage) and toughness (integral of the curve) can be determined. These data provide insight into the mechanical properties of the film. For the purposes of embodiments the differences in mechanical properties (toughness) between SOFs are denoted by their respective rupture points.

In embodiments, the rupture points of capped SOF films (with respect to the corresponding non-capped SOF compositions) may be attenuated by about 1% to about 85%, such as from about 5% to about 25%.

In embodiments, the rupture points of capped SOF films (with respect to the corresponding non-capped SOF compositions) may be enhanced by about 1% to about 400%, about 20% to about 200%, or from about 50% to about 100%.

In embodiments, the imaging members and/or photoreceptors of the present disclosure comprise an outermost layer that comprises a fluorinated SOF in which a first segment having hole transport properties, which may or may not be obtained from the reaction of a fluorinated building block, may be linked to a second segment that is fluorinated, such as a second segment that has been obtained from the reaction of a fluorine-containing molecular building block.

In embodiments, the fluorine content of the fluorinated SOFs comprised in the imaging members and/or photoreceptors of the present disclosure may be homogeneously distributed throughout the SOF. The homogenous distribution of fluorine content in the SOF comprised in the imaging members and/or photoreceptors of the present disclosure may be controlled by the SOF forming process and therefore the fluorine content may also be patterned at the molecular level.

In embodiments, the outermost layer of the imaging members and/or photoreceptors comprises an SOF wherein the microscopic arrangement of segments is patterned. The term "patterning" refers, for example, to the sequence in which segments are linked together. A patterned fluorinated SOF would therefore embody a composition wherein, for example, segment A (having hole transport molecule func-

tions) is only connected to segment B (which is a fluorinated segment), and conversely, segment B is only connected to segment A.

In embodiments, the outermost layer of the imaging members and/or photoreceptors comprises an SOF having only one segment, say segment A (for example having both hole transport molecule functions and being fluorinated), is employed is will be patterned because A is intended to only react with A.

10 In principle a patterned SOF may be achieved using any number of segment types. The patterning of segments may be controlled by using molecular building blocks whose functional group reactivity is intended to compliment a partner molecular building block and wherein the likelihood 15 of a molecular building block to react with itself is minimized. The aforementioned strategy to segment patterning is non-limiting.

In embodiments, the outermost layer of the imaging members and/or photoreceptors comprises patterned fluorinated SOFs having different degrees of patterning. For example, the patterned fluorinated SOF may exhibit full patterning, which may be detected by the complete absence 20 of spectroscopic signals from building block functional groups. In other embodiments, the patterned fluorinated SOFs having lowered degrees of patterning wherein domains of patterning exist within the SOF.

It is appreciated that a very low degree of patterning is associated with inefficient reaction between building blocks and the inability to form a film. Therefore, successful 30 implementation of the process of the present disclosure requires appreciable patterning between building blocks within the SOF. The degree of necessary patterning to form a patterned fluorinated SOF suitable for the outer layer of imaging members and/or photoreceptors can depend on the chosen building blocks and desired linking groups. The minimum degree of patterning required to form a suitable patterned fluorinated SOF for the outer layer of imaging members and/or photoreceptors may be quantified as formation of about 40% or more of the intended linking groups 35 or about 50% or more of the intended linking groups; the nominal degree of patterning embodied by the present disclosure is formation of about 80% or more of the intended linking group, such as formation of about 95% or more of the intended linking groups, or about 100% of the intended linking groups. Formation of linking groups may be detected spectroscopically.

In embodiments, the fluorine content of the fluorinated SOFs comprised in the outermost layer of the imaging members and/or photoreceptors of the present disclosure may be distributed throughout the SOF in a heterogeneous manner, including various patterns, wherein the concentration or density of the fluorine content is reduced in specific areas, such as to form a pattern of alternating bands of high and low concentrations of fluorine of a given width. Such patterning may be accomplished by utilizing a mixture of molecular building blocks sharing the same general parent molecular building block structure but differing in the degree of fluorination (i.e., the number of hydrogen atoms replaced with fluorine) of the building block.

60 In embodiments, the SOFs comprised in the outermost layer of the imaging members and/or photoreceptors of the present disclosure of the present disclosure may possess a heterogeneous distribution of the fluorine content, for example, by the application of highly fluorinated or perfluorinated molecular building block to the top of a formed wet layer, which may result in a higher portion of highly fluorinated or perfluorinated segments on a given side of the

SOF and thereby forming a heterogeneous distribution highly fluorinated or perfluorinated segments within the thickness of the SOF, such that a linear or nonlinear concentration gradient may be obtained in the resulting SOF obtained after promotion of the change of the wet layer to a dry SOF. In such embodiments, a majority of the highly fluorinated or perfluorinated segments may end up in the upper half (which is opposite the substrate) of the dry SOF or a majority of the highly fluorinated or perfluorinated segments may end up in the lower half (which is adjacent to the substrate) of the dry SOF.

In embodiments, comprised in the outermost layer of the imaging members and/or photoreceptors of the present disclosure may comprise non-fluorinated molecular building blocks (which may or may not have hole transport molecule functions) that may be added to the top surface of a deposited wet layer, which upon promotion of a change in the wet film, results in an SOF having a heterogeneous distribution of the non-fluorinated segments in the dry SOF. In such embodiments, a majority of the non-fluorinated segments may end up in the upper half (which is opposite the substrate) of the dry SOF or a majority of the non-fluorinated segments may end up in the lower half (which is adjacent to the substrate) of the dry SOF.

In embodiments, the fluorine content in the SOF comprised in the outermost layer of the imaging members and/or photoreceptors of the present disclosure may be easily altered by changing the fluorinated building block or the degree of fluorination of a given molecular building block. For example, the fluorinated SOF compositions of the present disclosure may be hydrophobic, and may also be tailored to possess an enhanced charge transport property by the selection of particular segments and/or secondary components.

In embodiments, the fluorinated SOFs may be made by the reaction of one or more molecular building blocks, where at least one of the molecular building blocks contains fluorine and at least one at least one of the molecular building blocks has charge transport molecule functions (or upon reaction results in a segment with hole transport molecule functions. For example, the reaction of at least one, or two or more molecular building blocks of the same or different fluorine content and hole transport molecule functions may be undertaken to produce a fluorinated SOF. In specific embodiments, all of the molecular building blocks in the reaction mixture may contain fluorine which may be used as the outermost layer of the imaging members and/or photoreceptors of the present disclosure. In embodiments, a different halogen, such as chlorine, and may optionally be contained in the molecular building blocks.

The fluorinated molecular building blocks may be derived from one or more building blocks containing a carbon or silicon atomic core; building blocks containing alkoxy cores; building blocks containing a nitrogen or phosphorous atomic core; building blocks containing aryl cores; building blocks containing carbonate cores; building blocks containing carbocyclic-, carbobicyclic-, or carbotricyclic core; and building blocks containing an oligothiophene core. Such fluorinated molecular building blocks may be derived by replacing or exchanging one or more hydrogen atoms with a fluorine atom. In embodiments, one or more one or more of the above molecular building blocks may have all the carbon bound hydrogen atoms replaced by fluorine. In embodiments, one or more one or more of the above molecular building blocks may have one or more hydrogen atoms replaced by a different halogen, such as by chlorine.

In addition to fluorine, the SOFs of the present disclosure may also include other halogens, such as chlorine.

In embodiments, one or more fluorinated molecular building blocks may be respectively present individually or 5 totally in the fluorinated SOF comprised in the outermost layer of the imaging members and/or photoreceptors of the present disclosure at a percentage of about 5 to about 100% by weight, such as at least about 50% by weight, or at least about 75% by weight, in relation to 100 parts by weight of the SOF.

In embodiments, the fluorinated SOF may have greater than about 20% of the H atoms replaced by fluorine atoms, such as greater than about 50%, greater than about 75%, greater than about 80%, greater than about 90%, or greater 15 than about 95% of the H atoms replaced by fluorine atoms, or about 100% of the H atoms replaced by fluorine atoms.

In embodiments, the fluorinated SOF may have greater than about 20%, greater than about 50%, greater than about 75%, greater than about 80%, greater than about 90%, 20 greater than about 95%, or about 100% of the C-bound H atoms replaced by fluorine atoms.

In embodiments, a significant hydrogen content may also be present, e.g. as carbon-bound hydrogen, in the SOFs of the present disclosure. In embodiments, in relation to the 25 sum of the C-bound hydrogen and C-bound fluorine atoms, the percentage of the hydrogen atoms may be tailored to any desired amount. For example the ratio of C-bound hydrogen to C-bound fluorine may be less than about 10, such as a ratio of C-bound hydrogen to C-bound fluorine of less than 30 about 5, or a ratio of C-bound hydrogen to C-bound fluorine of less than about 1, or a ratio of C-bound hydrogen to C-bound fluorine of less than about 0.1, or a ratio of C-bound hydrogen to C-bound fluorine of less than about 0.01.

In embodiments, the fluorine content of the fluorinated SOF comprised in the outermost layer of the imaging members and/or photoreceptors of the present disclosure may be of from about 5% to about 75% by weight, such as about 5% to about 65% by weight, or about 10% to about 40 50% by weight. In embodiments, the fluorine content of the fluorinated SOF comprised in the outermost layer of the imaging members and/or photoreceptors of the present disclosure is not less than about 5% by weight, such as not less than about 10% by weight, or not less than about 15% by weight, and an upper limit of the fluorine content is about 75% by weight, or about 60% by weight.

In embodiments, the outermost layer of the imaging members and/or photoreceptors of the present disclosure may comprise and SOF where any desired amount of the segments in the SOF may be fluorinated. For example, the percent of fluorine containing segments may be greater than about 10% by weight, such as greater than about 30% by weight, or greater than 50% by weight; and an upper limit percent of fluorine containing segments may be 100%, such as less than about 90% by weight, or less than about 70% by weight.

In embodiments, the outermost layer of the imaging members and/or photoreceptors of the present disclosure may comprise a first fluorinated segment and a second electroactive segment in the SOF of the outermost layer in an amount greater than about 80% by weight of the SOF, such as from about 85 to about 99.5 percent by weight of the SOF, or about 90 to about 99.5 percent by weight of the SOF.

In embodiments, the fluorinated SOF comprised in the outermost layer of the imaging members and/or photoreceptors of the present disclosure may be a “solvent resistant” SOF, a patterned SOF, a capped SOF, a composite SOF,

and/or a periodic SOF, which collectively are hereinafter referred to generally as an "SOF," unless specifically stated otherwise.

The term "solvent resistant" refers, for example, to the substantial absence of (1) any leaching out any atoms and/or molecules that were at one time covalently bonded to the SOF and/or SOF composition (such as a composite SOF), and/or (2) any phase separation of any molecules that were at one time part of the SOF and/or SOF composition (such as a composite SOF), that increases the susceptibility of the layer into which the SOF is incorporated to solvent/stress cracking or degradation. The term "substantial absence" refers for example, to less than about 0.5% of the atoms and/or molecules of the SOF being leached out after continuously exposing or immersing the SOF comprising imaging member (or SOF imaging member layer) to a solvent (such as, for example, either an aqueous fluid, or organic fluid) for a period of about 24 hours or longer (such as about 48 hours, or about 72 hours), such as less than about 0.1% of the atoms and/or molecules of the SOF being leached out after exposing or immersing the SOF comprising to a solvent for a period of about 24 hours or longer (such as about 48 hours, or about 72 hours).

The term "organic fluid" refers, for example, to organic liquids or solvents, which may include, for example, alkenes, such as, for example, straight chain aliphatic hydrocarbons, branched chain aliphatic hydrocarbons, and the like, such as where the straight or branched chain aliphatic hydrocarbons have from about 1 to about 30 carbon atoms, such as from about 4 to about 20 carbons; aromatics, such as, for example, toluene, xylenes (such as o-, m-, p-xylene), and the like and/or mixtures thereof; isopar solvents or isoparaffinic hydrocarbons, such as a non-polar liquid of the ISOPAR™ series, such as ISOPAR E, ISOPAR G, ISOPAR H, ISOPAR L and ISOPAR M (manufactured by the Exxon Corporation, these hydrocarbon liquids are considered narrow portions of isoparaffinic hydrocarbon fractions), the NORPART™ series of liquids, which are compositions of n-paraffins available from Exxon Corporation, the SOLTROL™ series of liquids available from the Phillips Petroleum Company, and the SHELLSOL™ series of liquids available from the Shell Oil Company, or isoparaffinic hydrocarbon solvents having from about 10 to about 18 carbon atoms, and or mixtures thereof. In embodiments, the organic fluid may be a mixture of one or more solvents, i.e., a solvent system, if desired. In addition, more polar solvents may also be used, if desired. Examples of more polar solvents that may be used include halogenated and nonhalogenated solvents, such as tetrahydrofuran, trichloro- and tetrachloroethane, dichloromethane, chloroform, monochlorobenzene, acetone, methanol, ethanol, benzene, ethyl acetate, dimethylformamide, cyclohexanone, N-methyl acetamide and the like. The solvent may be composed of one, two, three or more different solvents and/or and other various mixtures of the above-mentioned solvents.

Various exemplary embodiments encompassed herein include a method of imaging which includes generating an electrostatic latent image on an imaging member, developing a latent image, and transferring the developed electrostatic image to a suitable substrate.

While the description above refers to particular embodiments, it will be understood that many modifications may be made without departing from the spirit thereof. The accom-

panying claims are intended to cover such modifications as would fall within the true scope and spirit of embodiments herein.

The presently disclosed embodiments are, therefore, to be considered in all respects as illustrative and not restrictive, the scope of embodiments being indicated by the appended claims rather than the foregoing description. All changes that come within the meaning of and range of equivalency of the claims are intended to be embraced therein.

## EXAMPLES

The example set forth herein below and is illustrative of different compositions and conditions that can be used in practicing the present embodiments. All proportions are by weight unless otherwise indicated. It will be apparent, however, that the embodiments can be practiced with many types of compositions and can have many different uses in accordance with the disclosure above and as pointed out hereinafter.

To demonstrate the advantage of a hole transport molecule of the present embodiments, e.g., bis[4-(methoxymethyl)phenyl]phenylamine, the following prophetic examples were fabricated and described to demonstrate the feasibility of the present embodiments.

### Prophetic Example 1

#### Synthesis of a Fluorinated Structured Organic Film (FSOF) Containing Capping Units with Hole Transporting Properties

A FSOF solution is made by mixing a first building block 1H,1H,8H,8H-Dodecafluoro-1,8-octanediol; (7.49), a second building block TME-Ab118; (6.37); an anti-oxidant TrisTPM; (0.29 g). A capping unit HTM (4-(diphenylamino)phenyl)methanol (1.53 g), an acid catalyst delivered as 0.8 g of a 20 wt % solution of Nacure XP-357, a leveling additive delivered as 0.64 g of a 25 wt % solution of Silclean 3700, and 22.7 g of 1-methoxy-2-propanol.

The mixture is shaken and heated at 65° C. for 3 hours, which dissolves the solid constituents and reacts the building blocks together to form a structured network with capping units. The resulting mixture is then filtered through a 1 micron PTFE membrane and is tsukiagi cup coated onto a 40 mm drum photoreceptor and dried in a forced air oven at 155° C. for 40 minutes. The resulting cured FSOF overcoat layer is ~6 microns thick.

### Prophetic Example 2

A FSOF solution is made by mixing a first building block 1H,1H,8H,8H-Dodecafluoro-1,8-octanediol; (7.49), a second building block TME-Ab118; (6.37); an anti-oxidant TrisTPM; (0.29 g). A capping unit HTM 3-(phenyl(p-tolyl)amino)phenol (1.53 g), an acid catalyst delivered as 0.8 g of a 20 wt % solution of Nacure XP-357, a leveling additive delivered as 0.64 g of a 25 wt % solution of Silclean 3700, and 22.7 g of 1-methoxy-2-propanol.

The mixture is shaken and heated at 65° C. for 3 hours, which dissolves the solid constituents and reacts the building blocks together to form a structured network with capping units. The resulting mixture is then filtered through a 1 micron PTFE membrane and is tsukiagi cup coated onto a 40 mm drum photoreceptor and dried in a forced air oven at 155° C. for 40 minutes. The resulting cured FSOF overcoat layer is ~6 microns thick.

55

## Comparative Prophetic Example 3

A FSOF solution is made by mixing a first building block 1H,1H,8H,8H-Dodecafluoro-1,8-octanediol; (9.83 g), a second building block TME-Ab118; (9.41 g); an anti-oxidant 5 2,5-Di(tert-amyl) hydroquinone; (0.19 g) an acid catalyst delivered as 1.0 g of a 20 wt % solution of Nacure XP-357, a leveling additive delivered as 0.8 g of a 25 wt % solution of Siclean 3700, and 28.6 g of 1-methoxy-2-propanol.

The mixture is shaken and heated at 65° C. for 3 hours, 10 which dissolves the solid constituents and reacts the building blocks together to form a structured network with capping units. The resulting mixture is then filtered through a 1 micron PTFE membrane and is tsukiagi cup coated onto a 40 mm drum photoreceptor and dried in a forced air oven at 15 155° C. for 40 minutes. The resulting cured FSOF overcoat layer is ~6 microns thick.

## Comparative Prophetic Example 4

The base production photoreceptor used for Examples 1-3 having no overcoat layer is used for a comparative example.

## Electrical Evaluation

Comparative Example 4 with no overcoat layer is compared to Examples 1-3 on a Universal 40 mm drum electrical scanner set at 75 ms timing and having 680 nm exposure and erase. Photo-Induced-Discharge-Curves (PIDC) of all samples are taken and compared. Examples 1 and 2 show improved photo discharge compared to comparative Examples 3 and 4. This is thought to be due to the added capping units with hole transporting properties providing improved charge transport.

## Ghosting Evaluation

Comparative Example 3 without a capping unit is compared to Examples 1-2 by placing them in a Xerox Workcentre 7435 printer. Print testing is conducted in a stressful environment (A-zone: 28.degree.C., 85% RH) and using a known ghosting test pattern to evaluate image quality, specifically ghosting. Examples 1 and 2 show improved ghosting compared to comparative Examples 3. This is thought to be due to the added capping units with hole transporting properties providing improved charge transport.

All the patents and applications referred to herein are hereby specifically, and totally incorporated herein by reference in their entirety in the instant specification.

It will be appreciated that several of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. An imaging member comprising:

a substrate;

a charge generating layer;

a charge transport layer; and

an optional overcoat layer, wherein an outermost layer of

the imaging member comprises a structured organic

film (SOF) comprising:

molecular building blocks having a plurality of segments

and functional groups (Fg),

56

a plurality of linkers arranged as a covalent organic framework (COF), and

capping units for altering the mechanical and physical properties of the SOF via local interruption of the SOF framework, wherein the capping units comprise hole transport molecules bonding to more than 50% of the plurality of the functional groups (Fg), further wherein the hole transport molecules are selected from the group consisting of carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole); poly(vinylpyrene); poly(vinyltetraphene); poly(vinyltetracene); poly(vinylperylene); 2,4,7-trinitro-9-fluorenone; 2,4,5,7-tetranitro-fluorenone; dinitroanthracene; dinitroacridene; tetracyanopyrene; dinitroanthraquinone; butylcarbonylfluorenemalononitrile; bis(4-(methoxymethyl)phenyl)phenylamine, and mixtures thereof.

2. The imaging member of claim 1, wherein SOF includes a first fluorinated segment.

3. The imaging member of claim 2, wherein the first fluorinated segment is a segment comprising of:



4. The imaging member of claim 3, wherein the first fluorinated segment is obtained from a fluorinated building block selected from the group consisting of 2,2,3,3,4,4,5,5,5-octafluoro-1,6-hexanediol, 2,2,3,3,4,4,5,5,6,6,7,7-dodecanofluoro-1,8-octanediol, 2,2,3,3,4,4,5,5,6,6,7,7,8,8,9,9-perfluorodecane-1,10-dial, (2,3,5,6-tetrafluoro-4-hydroxymethyl-phenyl)-methanol, 2,2,3,3-tetrafluoro-1,4-butanediol, 2,2,3,3,4,4-hexafluoro-1,5-pentanediol, and 2,2,3,3,4,4,5,5,6,6,7,7,8,8-tetradecafluoro-1,9-nanediol.

5. The imaging member of claim 2, wherein the first fluorinated segment is present in the SOF of the outermost layer in an amount from about 25 to about 75 percent by weight of the SOF.

6. The imaging member of claim 1, wherein the capping unit is bonded to the framework of the SOF via a linker group.

7. The imaging member of claim 1, wherein the capping units to segment molar ratio in the SOF is from about 1:200 to about 1:3.

8. The imaging member of claim 1, wherein the capping units are distributed in a non-uniform manner within the SOF.

9. The imaging member of claim 1, wherein the charge transport layer is the outermost layer, and the charge transport layer is between from about 10 to about 40 microns thick.

10. The imaging layer of claim 1, wherein the charge generating layer and the charge transport layer are combined in a single layer with a thickness between about 10 to about 40 microns thick.

## 57

11. The imaging layer of claim 10, wherein the single layer is the outermost layer.

12. The imaging member of claim 1, wherein the SOF comprises a secondary component.

13. The imaging member of claim 12, wherein the secondary component is selected from the group consisting of conductivity agents, semiconductor agents, antioxidant agents, electron transport agents, hole transport agents, PTFE particles, and wax particles.

14. The imaging member of claim 1, wherein the capping units enhance an inclined or inherent property of the SOF.

15. The imaging member of claim 14, wherein the capping units enhance hole transport or electron transport in the SOF.

16. An imaging member comprising:

a substrate;

a charge generating layer;

a charge transport layer; and

an optional overcoat layer, wherein an outermost layer of

the imaging member comprises a structured organic film (SOF) comprising molecular building blocks having a plurality of segments including at least a first fluorinated segment and functional groups (Fg),

a plurality of linkers arranged as a covalent organic framework (COF),

capping units altering the mechanical and physical properties of the SOF via local interruption of the SOF framework, wherein the capping units comprise hole transport molecules bonding to more than 50% of the plurality of the functional groups (Fg) and a capping unit loading is greater than 5% by weight of the total weight of the SOF, and further wherein the hole transport molecules are selected from the group consisting of carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole);

poly(vinylpyrene); poly(vinyltetraphene); poly(vinyltetracene); poly(vinylperylene); 2,4,7-trinitro-9-fluorenone; 2,4,5,7-tetranitro-fluorenone; dinitroanthracene; dinitroacridene; tetracyanopyrene; dinitroanthraquinone; butylcarbonylfluorenemalononitrile; and mixtures thereof;

a charging unit to impart an electrostatic charge on the imaging member;

an exposure unit to create an electrostatic latent image on the imaging member;

an image material delivery unit to create an image on the imaging member;

a transfer unit to transfer the image from the imaging member; and

an optional cleaning unit.

18. The xerographic apparatus of claim 17, wherein the charging unit is selected from the group consisting of a biased charge roll and a scorotron.

## 58

dinitroanthracene; dinitroacridene; tetracyanopyrene; dinitroanthraquinone; butylcarbonylfluorenemalononitrile; and mixtures thereof.

17. A xerographic apparatus comprising:  
an imaging member, wherein an outermost layer of the imaging member comprises a structured organic film (SOF) comprising

molecular building blocks having a plurality of segments and functional groups (Fg),  
a plurality of linkers arranged as a covalent organic framework (COF),

capping units altering the mechanical and physical properties of the SOF via local interruption of the SOF framework, wherein the capping units comprise hole transport molecules bonding to more than 50% of the plurality of the functional groups (Fg), and further wherein the hole transport molecules are selected from the group consisting of carbazole; N-ethyl carbazole; N-isopropyl carbazole; N-phenyl carbazole; tetraphenylpyrene; 1-methylpyrene; perylene; chrysene; anthracene; tetraphene; 2-phenyl naphthalene; azopyrene; 1-ethyl pyrene; acetyl pyrene; 2,3-benzochrysene; 2,4-benzopyrene; 1,4-bromopyrene; poly(N-vinylcarbazole); poly(vinylpyrene); poly(vinyltetraphene); poly(vinyltetracene); poly(vinylperylene); 2,4,7-trinitro-9-fluorenone; 2,4,5,7-tetranitro-fluorenone; dinitroanthracene; dinitroacridene; tetracyanopyrene; dinitroanthraquinone; butylcarbonylfluorenemalononitrile; and mixtures thereof;

a charging unit to impart an electrostatic charge on the imaging member;

an exposure unit to create an electrostatic latent image on the imaging member;

an image material delivery unit to create an image on the imaging member;

a transfer unit to transfer the image from the imaging member; and

an optional cleaning unit.

\* \* \* \* \*